



US005223198A

# United States Patent [19]

Frankfort et al.

[11] Patent Number: 5,223,198

[45] Date of Patent: Jun. 29, 1993

[54] PROCESS OF MAKING MIXED SHRINKAGE YARN

[75] Inventors: Hans R. E. Frankfort, Greenville, N.C.; Benjamin H. Knox, Wilmington, Del.; James B. Noe, Wilmington, N.C.

[73] Assignee: E. I. Du Pont de Nemours and Company, Wilmington, Del.

[21] Appl. No.: 786,585

[22] Filed: Nov. 1, 1991

## Related U.S. Application Data

[63] Continuation-in-part of Ser. No. 338,251, Apr. 14, 1989, Pat. No. 5,066,447, which is a continuation-in-part of Ser. No. 53,309, May 22, 1987, abandoned, which is a continuation-in-part of Ser. No. 824,363, Jan. 30, 1986, abandoned.

[51] Int. Cl.<sup>5</sup> D02H 7/00; D02J 1/22

[52] U.S. Cl. 264/103; 28/172.2; 28/190; 264/210.8; 264/211.2; 264/235.6; 264/290.5

[58] Field of Search 264/103, 210.8, 211.12, 264/235.6, 290.5, 290.7; 28/172.2, 190

## References Cited

### U.S. PATENT DOCUMENTS

3,771,307 11/1973 Petrille 57/157 TS  
3,772,872 11/1973 Piazza et al. 57/140 R4,134,882 1/1979 Frankfort et al. .... 528/309  
4,156,071 5/1979 Knox ..... 528/272  
4,195,051 3/1980 Frankfort et al. .... 264/176 F  
4,407,767 10/1983 Seaborn ..... 264/40.1

## FOREIGN PATENT DOCUMENTS

3018373 11/1983 Fed. Rep. of Germany .  
3328449 2/1985 Fed. Rep. of Germany .

## OTHER PUBLICATIONS

F. Maag, Production of Warps From Flat Synthetic Filament Yarns, Textile Month, May 1984, pp. 48, 49, 50.

Frank Hunter, Draw-Bearing, Fiber World, Sep. 1984 pp. 61-68.

Primary Examiner—Leo B. Tentoni

[57]

## ABSTRACT

A process of making mixed shrinkage yarn, including drawing, especially cold-drawing, or hot-drawing or other heat-treatments of spin-oriented crystalline polyester filaments, and particularly polyester feed yarns, that have been prepared by spinning at speeds of, e.g., 4 km/min, and have low shrinkage and no natural draw ratio in the conventional sense, that provides useful technique for obtaining uniform drawn filaments of desired denier and of differential shrinkage, and thereby provides improved flexibility to obtain filaments and yarns of mixed shrinkage.

19 Claims, 15 Drawing Sheets



FIG.1



FIG.2



FIG. 3



FIG. 4



FIG. 5



FIG. 6



FIG. 8



FIG. 6



FIG. 10

YARN NO. VI-1



FIG. 11

YARN NO. VI-2



FIG.12

YARN NO. VI-3



FIG. 13  
YARN NO. VII-2



FIG. 14

YARN NO VIII-3



FIG. 15  
YARN NO IX-2



FIG. 16



YARN NO. VII-2

FIG. 17



YARN NO. IX-2

FIG. 18



FIG. 19



FIG.20



FIG. 21



PROCESS OF MAKING MIXED SHRINKAGE  
YARN

CROSS-REFERENCE TO RELATED  
APPLICATIONS

This is a continuation-in-part of application Ser. No. 07/338,251, filed by Knox and Noe Apr. 14, 1989; issued as U.S. Pat. No. 5066447, and which is sometimes referred to herein as the parent application, but is also itself a continuation-in-part application of application Ser. No. 07/053,309, filed May 2, 1987, as a continuation-in-part of application Ser. No. 824,363, filed Jan. 30, 1986 both abandoned.

TECHNICAL FIELD

This invention concerns improvements in and relating to polyester (continuous) filaments, especially in the form of filaments of differential shrinkage, and mixed shrinkage yarns thereof, and more especially to a capability to provide from the same feed stock such polyester continuous filament yarns of various differing deniers and shrinkages, as desired, and of other useful properties, including improved processes; and new polyester flat yarns, as well as filaments, generally, resulting from such processes, and downstream products from such filaments and yarns.

BACKGROUND OF PARENT APPLICATION

Textile designers are very creative. This is necessary because of seasonal factors and because the public taste continually changes, so the industry continually demands new products. Many designers in this industry would like the ability to custom-make their own yarns, so their products would be more unique, and so as to 35 provide more flexibility in designing textiles.

Polyester (continuous) filament yarns have for many years had several desirable properties and have been available in large quantities at reasonable cost, but, hitherto, there has been an important limiting factor in the usefulness of most polyester flat yarns to textile designers, because only a limited range of yarns has been available from fiber producers, and the ability of any designer to custom-make his own particular polyester flat yarns has been severely limited in practice. The fiber producer has generally supplied only a rather limited range of polyester yarns because it would be more costly to make a more varied range, e.g. of deniers per filament (dpf), and to stock an inventory of such different yarns.

Also, conventional polyester filaments have combinations of properties that, for certain end-uses, could desirably be improved, as will be indicated hereinafter. It is important to recognize that what is important for any particular end-use is the combination of all the properties of the specific yarn (or fiber), sometimes in the yarn itself during processing, but also in the eventual fabric or garment of which it is a component. It is easy, for instance, to reduce shrinkage by a processing treatment, but this modification is generally accompanied by other changes, so it is the combination or balance of properties of any filament (or staple fiber) that is important. Generally, hereinafter, we refer to flat (i.e., untextured) filament yarns. It will be recognized that, where appropriate, the technology may apply also to polyester filaments in other forms, such as tows, which may then be converted into staple fiber, and used as such in accordance with the balance of properties that is desirable

and may be achieved as taught hereinafter, but the advantage and need that the invention satisfies is more particularly in relation to flat filament yarns (i.e. untextured continuous filament yarns), as will be evident.

- 5 For textile purposes, a yarn must have certain properties, such as sufficiently high modulus and yield point, and sufficiently low shrinkage, which distinguish these yarns from feeder yarns that require further processing before they have the minimum properties for processing 10 into textiles and subsequent use. These feeder yarns are sometimes referred to as feed yarns, which is how we refer to them herein, for the most part. Conventionally, flat polyester filament yarns used to be prepared by melt-spinning at low speeds (to make undrawn yarn that 15 is sometimes referred to as LOY) and then drawing and heating to reduce shrinkage and to increase modulus and yield point.

It has long been known that such undrawn (LOY) polyester filaments draw by a necking operation, as 20 disclosed by Marshall and Thompson in J. Applied Chem., 4, (April 1954), pp. 145-153. This means that the undrawn polyester filaments have a natural draw ratio. Drawing such polyester filaments has not been generally desirable (or practiced commercially) at draw ratios less than this natural draw ratio because the result 25 has been partial-drawing (i.e., drawing that leaves a residual elongation of more than about 30% in the drawn yarns) that has produced irregular "thick-thin" filaments which have been considered inferior for most practical commercial purposes (unless a specialty yarn 30 has been required, to give a novelty effect, or special effect). For filament yarns, the need for uniformity is particularly important, more so than for staple fiber. Fabrics from flat (i.e. untextured) yarns show even minor differences in uniformity from partial drawing of conventional undrawn polyester yarns as defects, especially when dyeing these fabrics. Thus, uniformity in flat filament yarns is extremely important. The effect of 40 changing the draw ratio within the partial-draw-range of draw ratios (below the natural draw ratio) has previously had the effect of changing the proportions of lengths of drawn and undrawn filament in previous products. Thus, hitherto it has not been possible to obtain from the same LOY feed yarn two satisfactory different uniform yarns whose deniers per filament (dpf) have varied from each other's by as much as 10%, because one of such yarns would have been non-uniform (or filaments would have broken to an unacceptable extent).

Undrawn polyester filaments have been unique in this respect because nylon filaments and polypropylene filaments have not had this defect. Thus, it has been possible to take several samples of a nylon undrawn 55 yarn, all of which have the same denier per filament, and draw them, using different draw ratios, to obtain correspondingly different deniers in the drawn yarns, as desired, without some being irregular thick-thin yarns, like partially drawn polyester filaments. This is pertinent to a relatively new process referred to variously as "warp-drawing", "draw-warping" or "draw-beaming", as will be evident herein.

For many textile processes, such as weaving and warp knitting, it has been customary to provide textile yarns in the form of warp yarns carefully wound on a large cylinder referred to as a beam. A beaming operation has always involved careful registration and winding onto the beam of warp yarns provided from a large

creel. Formerly, the warp yarns on the creel used to be drawn yarns, already suitable for use in textile processes, such as weaving and knitting.

Recently, there has been interest in using flat undrawn filament yarns, which have generally been cheaper than drawn yarns, and incorporating a drawing step in the beaming operation, as disclosed, e.g., by Seaborn, U.S. Pat. No. 4,407,767. This process is referred to herein as "draw-warping", but is sometimes called draw-beaming or warp-drawing. At least three commercial draw-warping machines have been offered commercially. Barmag/Liba have cooperated and built a unit, which is described and illustrated in *Chemiefasern/Textilindustrie*, February 1985, page 108 and pp. E14-15. There are also articles in *Textile Month*, March 1985, page 17, and in *Textile World*, May 1985, page 53. Karl Mayer/Dienes sell commercial draw-beaming systems, as advertised, e.g., on page 113 of the same February 1985 issue of *Chemiefasern/Textilindustrie*. The concept was discussed by Frank Hunter in *Fiber World*, September 1984, pages 61-68, in an article entitled "New Systems for Draw-Beaming POY Yarns", with reference to the Liba/Barmag and Karl Mayer systems using polyester POY and nylon. The Karl Mayer system was also described by F. Maag in *Textile Month*, May 1984, pages 48-50. Karl Mayer also have patents, e.g., DE 3,018,373 and 3,328,449. Cora/Val Lesina have also been selling draw-warping systems for some time, and have patents pending. These commercial machines are offered for use with polyester, polyamide or polypropylene yarns, the drawing systems varying slightly according to the individual yarns. As indicated, the object is to provide beams of drawn warp yarns, that are essentially similar to prior art beams of warp yarns, but from undrawn feed yarns. The advantages claimed for draw-warping are set out, e.g., in the article by Barmag/Liba, and have so far been summarized as better economics and better product quality.

As indicated, draw-warping had been suggested and used for polyester yarns. The article by Barmag/Liba indicates that POY, MOY or LOY yarn packages can be used to cut the raw material costs. POY stands for partially oriented yarn, meaning spin-oriented yarn spun at speeds of, e.g., 3-4 km/min for use as feeder yarns for draw-texturing. Huge quantities of such feeder yarns have been used for this purpose over the past decade, as suggested in Petrille, U.S. Pat. No. 3,771,307 and Piazza & Reese, U.S. Pat. No. 3,772,872. These draw-texturing feeder yarns (DTFY) had not been used, e.g., as textile yarns, because of their high shrinkage and low yield point, which is often measurable as a low  $T_7$  (tenacity at 7% elongation) or a low modulus (M). In other words, POY used as DTFY is not "hard yarn" that can be used as such in textile processes, but are feeder yarns that are drawn and heated to increase their yield point and reduce their shrinkage. MOY means medium oriented yarns, and are prepared by spinning at somewhat lower speeds than POY, e.g., 2-2.5 km/min, and are even less "hard", i.e., they are even less suitable for use as textile yarns without drawing. LOY means low oriented yarns, and are prepared at much lower spinning speeds of the order of 1 km/min or much less.

As has already been explained above and by Marshall and Thompson, conventional undrawn LOY polyester has a natural draw ratio. Attempts at "partial drawing" at lower draw ratios (such as leave a residual elongation of more than about 30% in the drawn yarns) will gener-

ally produce highly irregular "thick-thin" filaments, which are quite unsuitable for most practical commercial purposes. Among other important disadvantages, this severely limits the utility of LOY polyester as a practical draw-warping feed yarn. When undrawn polyester draw-texturing feed yarns of high shrinkage are prepared at higher spinning speeds, there is still generally a natural draw ratio at which these yarns prefer to be drawn, i.e., below which the resulting yarns are irregular; although the resulting irregularity becomes less noticeable, e.g., to the naked eye or by photography, as the spinning speed of the precursor feed yarns is increased, the along-end denier variations of the partial drawn yarns are nevertheless greater than are commercially desirable, especially as the resulting fabrics or yarns are generally dyed. Yarn uniformity is often referred to in terms of % Uster, or can be expressed as Denier Spread, as will be discussed hereinafter. It is not merely a question of denier uniformity, although this may be a convenient check on whether a yarn is uniform, as partially-drawn denier variations often mean the filaments have not been uniformly oriented along-end, and variations in orientation affect dye-uniformity. Dyeing uniformity is very sensitive to variations resulting from partial drawing. So, even for polyester POY prepared at relatively high spinning speeds, as will be seen hereinafter in the Example, partial drawing of such POY has produced yarn that is unacceptable, e.g., from a dyeing uniformity standpoint. Thus, hitherto, even with POY, such as has been used as feed yarn for draw-texturing (often referred to as DTFY herein), it has not been practical to draw-warp the same such POY (DTFY) to two different dpfs that vary from each other by as much as 10% and obtain two satisfactory uniform drawn yarns without significant broken filaments, because one would have been partially drawn.

Thus, it will be understood that a serious commercial practical defect of prior suggestions for draw-warping most prior undrawn polyester (POY, MOY or LOY) had been the lack of flexibility in that it had not been possible to obtain satisfactory uniform products using draw ratios below the natural draw ratio for the polyester feed yarn. This was different from the situation with nylon POY or polypropylene.

So far as is known, it had not previously been suggested that a draw-warping process be applied to a polyester textile yarn, i.e., one that was itself already a direct-use yarn, such as had shrinkage properties that made it suitable for direct use in textile processes such as weaving and knitting without first drawing. Indeed, to many skilled practitioners, it might have seemed a contradiction in terms to subject such a yarn to draw-warping because such a yarn was already a textile yarn, not a feed yarn that needed a drawing operation to impart properties useful in textile processes such as weaving or knitting.

According to the parent application (Ser. No. 07/338,251 referred to hereinabove, the disclosure of which is hereby incorporated herein by reference), processes were provided for improving the properties of feed yarns of undrawn polyester filaments. Such processes involved drawing with or without heat during the drawing and with or without post heat-treatment, and are most conveniently adapted for operation using a draw-warping machine, some such being sometimes referred to as draw-beaming or warp-drawing operations.

Preferred undrawn polyester feed yarns comprise spin-oriented polyester filaments of low shrinkage, such as have been disclosed in Knox U.S. Pat. No. 4,156,071. Alternatively, spin-oriented feed yarns of low shrinkage may be prepared at speeds higher than are used in the Knox patent, including speeds and conditions such as are disclosed by Frankfort & Knox in U.S. Pat. Nos. 4,134,882 and 4,195,051.

From time to time, interest has been shown in making filaments of differential shrinkage, especially from one 10 and the same filament feed stock, and especially for making mixed shrinkage filament yarns.

Over the years many prior suggestions have been made, but the suggestions have had technical disadvantages and have sometimes been costly, so far as commercial manufacture would have been concerned. Also, it is important to maintain uniformity, both along-end and between the various filaments. Lack of uniformity often shows up in the eventual dyed fabrics as dyeing defects, so is undesirable.

The present invention provides a technique by which mixed shrinkage polyester filament yarns may be made efficiently, from the same feed stock if desired, and without some of the cost disadvantages referred to above. This may be achieved by use of the same feed 25 yarns as for the parent application, and adapting the processing of some of the filaments to provide the desired difference in shrinkage. Alternatively, mixed shrinkage may be provided by co-mingling filaments of high shrinkage, such as conventional polyester POY, 30 with spin-oriented low shrinkage polyester filaments, such as are used for feed yarns in the parent application. For convenience herein the former filaments of high shrinkage are referred to as (A<sub>F</sub>), whereas the low shrinkage filaments are referred to as (B<sub>F</sub>). These filaments may be processed and co-mingled as described 35 herein to provide mixed shrinkage yarns.

#### SUMMARY OF THE INVENTION

According to the present invention, there are provided the following processes:

A process for improving the properties of a mixed shrinkage yarn of spin-oriented polyester filaments of elongation-to-break (E<sub>B</sub>) about 40 to about 120% comprised of polyester filaments (A<sub>F</sub>) of high boil-off 45 shrinkage (S<sub>1</sub>) greater than about 15% and of low shrinkage polyester filaments (B<sub>F</sub>), characterized in that the mixed shrinkage yarn is cold-drawn without heat-setting to provide drawn filaments of elongation-to-break (E<sub>B</sub>) less than about 30% from drawing said filaments (A<sub>F</sub>) of high boil-off shrinkage, and wherein said 50 low shrinkage filaments (B<sub>F</sub>) are of tenacity at 7% elongation (T<sub>7</sub>) at least about 0.7 grams/denier, boil-off shrinkage (S<sub>1</sub>) less than about 10%, thermal stability as shown by an (S<sub>2</sub>) value less than about +1%, net shrinkage (S<sub>12</sub>) less than about 8%, maximum shrinkage tension (ST) less than about 0.3 grams/denier, density (ρ) about 1.35 to about 1.39 grams/cubic centimeter, and crystal size (CS) about 55 to about 90 Angstroms and also at least about (250ρ-282.5) Angstroms.

Such a mixed shrinkage yarn is preferably prepared by cospinning polyester filaments (A<sub>F</sub>) and (B<sub>F</sub>) and winding said mixed shrinkage yarn at a speed of at least 3.5 xm/min.

A process for preparing a mixed shrinkage yarn, 65 wherein spin-oriented polyester filaments (A<sub>F</sub>) of elongation-to-break (E<sub>B</sub>) about 40 to 120% and of high boil-off shrinkage (S<sub>1</sub>) greater than about 15% are cold-

drawn without heat-setting to provide drawn filaments of elongation-to-break (E<sub>B</sub>) less than about 30%, and spin-oriented low shrinkage polyester filaments (B<sub>F</sub>) are cold-drawn without heat setting and the filaments are co-mingled before or after drawing to form a mixed shrinkage yarn, and wherein said filaments (B<sub>F</sub>) are of elongation-to-break about 40 to about 120% tenacity at 7% elongation (T<sub>7</sub>) at least about 0.7 grams/denier, boil-off shrinkage (S<sub>1</sub>) less than about 10%, thermal stability as shown by an (S<sub>2</sub>) value less than about +1%, net shrinkage (S<sub>12</sub>) less than about 8%, maximum shrinkage tension (ST) less than about 0.3 grams/denier, density (ρ) about 1.35 to about 1.39 grams/cubic centimeter, and crystal size (CS) about 55 to about 90 Angstroms and also at least about (250ρ-282.5) Angstroms.

A process for preparing a mixed shrinkage yarn, wherein spin-oriented polyester filaments (A<sub>F</sub>) of high boil-off shrinkage (S<sub>1</sub>) greater than about 15% are cold-drawn without post heat treatment, said drawing being 20 carried out such that the elongation-to-break (E<sub>B</sub>) of the resulting drawn filaments is less than about 30%, and spin-oriented low shrinkage polyester filaments (B<sub>F</sub>) are drawn hot, with or without post heat treatment, and the resulting drawn filaments are co-mingled to provide a mixed shrinkage yarn of uniformly drawn filaments, wherein said low shrinkage filaments (B<sub>F</sub>) are of elongation-to-break (E<sub>B</sub>) about 40 to about 120%, tenacity at 7% elongation (T<sub>7</sub>) at least about 0.7 grams/denier, boil-off shrinkage (S<sub>1</sub>) less than about 10%, thermal stability as shown by an (S<sub>2</sub>) value less than about +1%, net shrinkage (S<sub>12</sub>) less than about 8%, maximum shrinkage tension (ST) less than about 0.3 grams/denier, density (ρ) about 1.35 to about 1.39 grams/cubic centimeter, and crystal size (CS) about 55 to about 90 Angstrom and also at least about (250ρ-282.5) Angstroms.

A process for preparing a mixed shrinkage yarn, wherein spin-oriented polyester filaments (A<sub>F</sub>) of high boil-off shrinkage (S<sub>1</sub>) greater than about 15% and spin-oriented low shrinkage polyester filaments (B<sub>F</sub>) are cold-drawn to form separate drawn filament bundles (A<sub>D</sub>) and (B<sub>D</sub>), respectively, and such that the elongation-to-break (E<sub>B</sub>) of resulting drawn filament bundle (A<sub>D</sub>) is less than about 30%, and one bundle is heat set and co-mingled with the other bundle to provide a mixed shrinkage yarn of uniformly drawn polyester filaments, and wherein said low shrinkage filaments (B<sub>F</sub>) are of elongation-to-break (E<sub>B</sub>) about 40 to about 120%, tenacity at 7% elongation (T<sub>7</sub>) at least about 0.7 grams/denier, boil-off shrinkage (S<sub>1</sub>) less than about 10%, thermal stability as shown by an (S<sub>2</sub>) value less than about +1%, net shrinkage (S<sub>12</sub>) less than about 8%, maximum shrinkage tension (ST) less than about 0.3 grams/denier, density (ρ) about 1.35 to about 1.39 grams/cubic centimeter, and crystal size (CS) about 55 to about 90 Angstrom and also at least about (250ρ-282.5) Angstroms.

A process for preparing a mixed shrinkage yarn, wherein spin-oriented polyester filaments (A<sub>F</sub>) of high boil-off shrinkage (S<sub>1</sub>) greater than about 15% are 60 drawn hot, with or without post heat treatment, such that the elongation-to-break (E<sub>B</sub>) of the resulting drawn filaments is less than about 30%, and spin-oriented low shrinkage polyester filaments (B<sub>F</sub>) are drawn cold, without post heat treatment, and the resulting drawn filaments are co-mingled to provide a mixed shrinkage yarn of uniformly drawn polyester filaments, wherein said low shrinkage filaments (B<sub>F</sub>) are of elongation-to-break (E<sub>B</sub>) about 40 to about 120%, tenacity at 7%

elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter, and crystal size (CS) about 55 to about 90 Angstroms and also at least about (250 $\rho$ -282.5) Angstroms.

A process for preparing a mixed shrinkage yarn, wherein spin-oriented polyester filaments ( $A_F$ ) of high boil-off shrinkages ( $S_1$ ) greater than about 15% are cold-drawn with or without heat setting, said drawing being carried out such that the elongation-to-break ( $E_B$ ) of the resulting drawn filaments is less than about 30%, and co-mingled with spin-oriented low shrinkage polyester filaments ( $B_F$ ) to provide a mixed shrinkage yarn, and wherein said low shrinkage filaments ( $B_F$ ) are of elongation-to-break ( $E_B$ ) about 40 to 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter, and crystal size (CS) about 55 to about 90 Angstroms and also at least about (250 $\rho$ -282.5) Angstroms.

A process for preparing a mixed shrinkage yarn, characterized in that spin-oriented polyester filaments are cold-drawn, the resulting drawn filaments are separated into at least two filament bundles, only one of which bundles is heat set, and then the filament bundles are co-mingled to provide a mixed shrinkage yarn of uniformly drawn filaments, wherein said spin-oriented filaments are of elongation-to-break ( $E_B$ ) about 40 to about 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter, and crystal size (CS) about 55 to about 90 Angstroms and also at least about (250 $\rho$ -282.5) Angstroms.

A process for preparing a mixed shrinkage yarn from at least two bundles of low shrinkage spin-oriented polyester filaments, wherein one of said bundles is drawn cold without post heat treatment and another of said bundles is drawn hot or cold with post heat treatment, or drawn hot with post heat treatment, and the resulting drawn filaments are co-mingled to provide a mixed shrinkage yarn of uniformly drawn filaments, and wherein said spin-oriented filaments are of elongation-to-break ( $E_B$ ) about 40 to about 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter, and crystal size (CS) about 55 to about 90 Angstroms and also at least about (250 $\rho$ -282.5) Angstroms.

A process for preparing a mixed shrinkage yarn from at least two bundles of low shrinkage spin-oriented polyester filaments, wherein one of said bundles is drawn hot with or without post heat treatment and the resulting drawn filaments are comingled with another of said bundles of spin-oriented filaments to provide a mixed shrinkage yarn, and wherein said spin-oriented

filaments are of elongation-to-break ( $E_B$ ) about 40 to about 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter, and crystal size (CS) about 55 to about 90 Angstroms and also at least about (250 $\rho$ -282.5) Angstroms.

Thus, the invention contemplates a process for preparing a mixed shrinkage yarn with filaments of higher shrinkage and filaments of lower shrinkage wherein the filaments of lower shrinkage are undrawn polyester filaments ( $B_F$ ), as aforesaid, that are processed with or without post heat treatment.

The undrawn polyester filaments preferably have an elongation ( $E_B$ ) about 60 to about 90%.

The drawing may, if desired, be carried out in the form of a weftless warp sheet of yarns and/or filament bundles prior to knitting, weaving or winding onto a beam.

The resulting mixed shrinkage yarns are also provided, according to the present invention, and preferably have a differential filament shrinkage of at least about 5% and a maximum shrinkage tension (ST) at least about 0.15 gpd, and the filaments and/or yarns may, if desired, be air jet-textured to provide textured yarns.

The bulk in the yarn is developed conveniently by appropriate heat treatment, on account of the difference in shrinkage of the component filaments, and such a process is provided according to the invention. Conveniently, such bulky filament bundles may be developed by heat relaxation of the filament bundles in the form of a weftless warp sheet, if desired.

Polyester polymers, used herein, may, if desired, be modified by incorporating ionic dye sites, such as ethylene-5-M-sulfo-isophthalate residues, where M is an alkali metal cation, for example in the range of about 1-3 mole % ethylene-5-sodium-sulfo-isophthalate residues, to provide dyeability with cationic dyes, as disclosed by Griffing and Remington in U.S. Pat. No. 3,018,272. A suitable polymer of relative viscosity (LRV) about 13 to about 18 is particularly useful. Representative copolymers used herein to enhance dyeability with disperse dyes are described in part by Most U.S. Pat. No. 4,444,710, Pacofsky U.S. Pat. No. 3,748,844, Hancock U.S. Pat. No. 4,639,347, and Frankfort and Knox U.S. Pat. Nos. 4,134,882 and 4,195,051, and representative chainbranching agents used herein to reduce shrinkage, especially of polyesters modified with ionic dye sites and/or copolymers, are described in part in Knox U.S. Pat. No. 4,156,071, MacLean U.S. Pat. No. 4,092,229, and Reese U.S. Pat. Nos. 4,883,032; 4,996,740; and 5,034,174. To obtain undrawn feed yarns of low shrinkage from modified polyesters, it is generally advantageous to increase polymer viscosity by about +0.5 to about +1.0 LRV units and/or add minor amounts of chainbranching agents (e.g., about 0.1 mole percent).

Advantageously, if desired, mixed shrinkage yarns may be prepared according to the invention from undrawn feed yarns that have been treated with caustic in the spin finish (as taught by Grindstaff and Reese in copending allowed patent application Ser. No. 07/420,459, filed Oct. 12, 1989) to enhance their hydrophilicity and provide improved moisture-wicking and

comfort. Incorporating filaments of different deniers and/or cross-sections may also be used to reduce filament-to-filament packing and thereby improve tactile aesthetics and comfort. Unique dyeability effects may be obtained by co-mingling drawn filaments of differing polymer modifications, such as homopolymer dyeable with disperse dyes and ionic copolymers dyeable with cationic dyes.

#### BRIEF DESCRIPTION OF DRAWINGS

FIG. 1 shows schematically a typical commercial draw-warping machine that may be used to practice a preferred process of the invention.

FIGS. 2-6 are graphs.

FIGS. 7-9 compare along-end denier Uster traces.

FIGS. 10-12 are curves showing load plotted v. elongation (-to-break).

FIGS. 13-15 are more along-end denier Uster traces.

FIGS. 16 and 17 are photographs of dyed fabrics.

FIGS. 18-20 are more curves showing load plotted v. elongation.

FIG. 21 is a plot of boil-off shrinkage ( $S_1$ ) and shrinkage tension (ST) v. spin speed.

#### DETAILED DESCRIPTION

Much of the description herein, for convenience, follows that in the parent application, and is followed by "MIXED SHRINKAGE EXAMPLES" that disclose ways of obtaining mixed shrinkage yarns according to the present invention.

Many of the parameters and measurements mentioned herein are fully discussed and described in the aforesaid Knox patent and in the Frankfort & Knox patents, all of which are hereby specifically incorporated herein by reference, so further detailed discussion herein would, therefore, be redundant. Such parameters include the tensile, shrinkage, orientation (birefringence), crystallinity (density and crystal size), viscosity and dye-related measurements, except in so far as mentioned and/or modified hereinafter.

Preferred polyester feed yarn filaments are undrawn in the sense disclosed by Knox, Frankfort & Knox, Petrille and Piazza & Reese. The feed yarn filaments are referred to as spin-oriented, because the orientation (and crystallization eventually derived therefrom) is caused by high-speed spinning, as opposed to the older process of first spinning at low speeds, of the order 0.5 (or as much as 1) km/min, to make LOY, followed by drawing and annealing which older process produces a completely different crystal fine structure in such conventional drawn yarns, in contrast to the combination of lower orientation and larger crystals derived from high-speed spinning (spin-orientation). This combination provides many advantages, such as improved dyeability and shrinkage properties, as disclosed by Knox and by Frankfort & Knox.

A low shrinkage is an essential requirement for textile yarns, as discussed by Knox; in fact, the shrinkage behavior of conventional drawn polyester yarns has not been as good as for other yarns, e.g., cellulose acetate, and this has caused textile manufacturers to use correspondingly different techniques for polyester fabric construction and finishing. At relatively high spinning speeds, e.g., as described by Frankfort & Knox, of the order of 5 km/min and higher, it is difficult to obtain uniform filaments without the desired low shrinkage under preferred spinning conditions. However, at speeds of the order of 4 km/min, as disclosed by Knox,

special spinning conditions are necessary to prepare the preferred feed yarns of low shrinkage and having the other requirements of uniformity and tensile properties. In contrast, POY has lower crystallinity and significantly higher shrinkage such as is desired for use as feeder yarns for draw-texturing, this having been a very much larger end-use than direct-use untextured polyester filament yarn. It becomes increasingly difficult to obtain extremely low shrinkage values in undrawn polyester yarns directly by high speed spinning, and so the preferred feed yarns will, in practice, rarely have  $S_1$  below about 2%, although this may be desirable.

The shrinkage and shrinkage tension measurements were as measured in U.S. Pat. No. 4,156,071, except that

15 the loads were 5 mg/denier for 30 minutes when measuring  $S_1$  (boil-off shrinkage), and for 3 minutes at 350° F. (177° C.) for  $S_2$  and DHS, to simulate trade heat-set conditions. The thermal stability ( $S_2$ ) is a measure of the additional change in length on exposure to dry heat (350° F.) after initial boil-off shrinkage ( $S_1$ ). The feed yarns of this invention have  $S_2$  values of less than about +1%, i.e., the yarns do not shrink significantly during the test. Under the test conditions, some yarns may elongate, in which case the  $S_2$  value is given in a parenthesis. The feed yarns generally do not elongate more than about 3%. The drawn yarns of this invention have  $S_2$  values of less than about +2% (i.e., shrink less than about 2%) and generally do not elongate greater than about 3%. The net shrinkage is the sum of  $S_1$  and  $S_2$ , 30 accordingly, is designated  $S_{12}$ ; although this has not often been referred to in the literature, it is a very important value, in some respects, for the fabric manufacturer, since a high and/or non-uniform net shrinkage ( $S_{12}$ ) means an important loss in effective fabric dimensions, as sold to the eventual consumer. Uniformity of shrinkage is also not often referred to, but is often very important in practice in fabric formation. The drawn filaments of the present invention show an important advantage over conventional polyester in this respect.

40 The combination of low shrinkage values ( $S_1$ ,  $S_2$  and  $S_{12}$ ) of the feed yarns used in the process of the invention (hereinafter the feed yarns) distinguishes such feed yarns from conventional POY, which as DTFY, i.e. as a feeder yarn for draw-texturing, preferably has low crystallinity and so higher shrinkage, and from conventional drawn yarns. Preferably the feed yarns have both  $S_1$  and  $S_{12}$  values less than about 6%.

As indicated hereinbefore, it is very surprising that the feed yarns can be fully or partially cold-drawn uniformly, in other words to provide drawn yarns/filaments of uniform denier (along-end), in contrast to the less satisfactory results of cold-drawing conventional undrawn polyester filaments. The ability to fully or partially draw by cold-drawing polyester filaments according to the present invention to provide uniformly drawn filaments is an important advantage, since this makes it possible to improve tensiles without a drastic reduction in dyeability or increase in shrinkage, and thus provide yarns, filaments and tows with an improved combination of tensiles, dyeability and shrinkage. This cold-drawing does increase the low shrinkage values of the feed yarns, and there is some reduction in the easy dyeability, these being such notable advantages of the feed yarns (in contrast to conventional polyester), and this is a good example of the need to consider the total combination (or balance) of properties of any polyester filaments or yarns, rather than a single property in isolation. However, even this combination of increased

shrinkage and reduced dyeability of the resulting drawn yarns is still generally significantly improved over conventional drawn polyester, because of the different crystal fine structure that results from spin-orientation, and consequent crystallization. The low shrinkage values, especially  $S_{12}$ , distinguish the drawn products, i.e., filaments, yarns and tows (and staple therefrom) of the invention from conventional drawn polyester. Preferably, these drawn products have both  $S_1$  and  $S_{12}$  values less than about 6%.

In some end-uses, a low shrinkage tension is very important because less tension is generated during yarn processing, and later, in fabrics, less puckering occurs, in contrast to drawn yarns. A preferred value for both feed yarns and drawn products is less than 0.15 grams/-denier.

Of the tensile measurements, only the post yield modulus (PYM) requires explanation and definition, as follows, and as illustrated with reference to FIGS. 2 and 3, which are both graphs plotting stress ( $\sigma$ ) against elongation (E) for a preferred feed yarn, FIG. 2, and a resulting drawn yarn, FIG. 3. The stress ( $\sigma$ ) at any elongation (E) which is measured as a percentage of the original length) is given in grams/denier by:

$$\text{Stress } (\sigma) = 0.01(100 + E) \times (\text{Load/initial denier}).$$

Thus the stress is calculated in terms of the denier at the time of measurement (which denier changes during elongation) whereas the tenacity is usually recorded in terms of the initial denier only. If a yarn has a yield zone, as shown in FIG. 2, this will be clear on a plot of stress v. E. The yield zone ( $E''-E'$ ) is the range of elongation for which the stress first decreases and then increases below  $\sigma_y$ , i.e., when the yarn yields because the stress decreases below peak value  $\sigma_y$  as E increases beyond  $E'$  (when  $\sigma$  passes through peak value  $\sigma'y$ ) until the stress again regains peak value  $\sigma'y$  at  $E''$  (the post-yield point). As indicated hereinbefore, preferred feed yarns were described by Knox, and have advantages in some end-uses (somewhat like cellulose acetate) partly because of their relatively low modulus. This advantage in aesthetics is however accompanied by a relatively low yield point (shown by a relatively large yield zone) which can be a disadvantage if it is desirable to use such yarns as filling, because the sudden increases in stress imposed by many weaving techniques may stretch such yarns irreversibly and only intermittently, with a resulting defect that can be revealed when the woven fabric is later dyed.

It is surprising that the feed yarns which, according to the invention, show a distinct yield zone,  $E''-E' > 0$ , in the plot of Stress v. E, so that there is a natural draw ratio in this sense looking at the plot, but such feed yarns do not perform as if there is a natural draw ratio when drawn at lower draw ratios, since such preferred feed yarns draw uniformly at such low draw ratios, in contrast to conventional POY spun at similar speeds but of higher shrinkage.

The post yield modulus is defined herein as the slope of the plot of stress v. elongation between  $E_7$  and  $E_{20}$ , i.e., elongations of 7 and 20%, and is given by the relationship:

$$\text{PYM} = \frac{\sigma_{20} - \sigma_7}{E_{20} - E_7}$$

However, since generally one records load/initial denier; rather than stress, PYM is always calculated herein according to the following equivalent relationship:

$$\text{PYM} = \frac{1.2 T_{20} - 1.07 T_7}{0.13}$$

The  $\sqrt{\text{PYM}}$  after boil-off (ABO) should be in the approximate range 2.5 to 5, preferably 3 to 5, corresponding to absence of any yield zone.

Reverting to the feed yarns, the minimum value of  $T_7$  (0.7 g/d) and the range of  $E_B$  (40-120%) coupled with large crystals, are important characteristics of spin-oriented yarns that provide the ability to be drawn uniformly as indicated above, in contrast with conventional POY and other undrawn yarns of higher shrinkage which are not capable of consistent drawing at low draw ratios to provide filaments of equivalent uniformity. Such combination of parameters approximates to a yield zone of less than 15%. Preferably the  $T_7$  is at least 0.8 g/d, and the  $E_B$  is less than 90%, corresponding to a yield zone of less than 10%. In practice,  $T_7$  is not usually greater than 17 g/d for feed yarns, and more usually less than about 1.2 g/d. Drawing increases the  $T_7$ , the preferred minimum of  $T_7$  is about 1 g/d, with  $E_B$  about 20-90%, and preferably about 20-60%, which provides sufficient initial tensiles for textile processability, even for weaving. Thus, by drawing, especially by cold-drawing, it is possible to improve the tensiles (and textile processability) of preferred feed yarns so that they can sustain sudden stresses such as are encountered for filling yarns in weaving processes, without impairing the uniformity, or losing all the advantages of improved dyeability and better shrinkage properties than conventional drawn polyester yarn. Preferred tenacity (T), and modulus (M), values in g/d, respectively, are at least 2.5, and in the range 40-100 for the drawn yarns, which provide useful textile properties with a wider range of fabric textile aesthetics than available with conventional drawn polyester. These drawn yarns are "hard yarns" with essentially no yield zone, unlike preferred precursor feed yarns, as shown by the range of  $\sqrt{\text{PYM}}$  (ABO) mentioned above.

Although the process of the invention is not limited to cold-drawing, the importance of the ability for the first time to carry out cold-drawing (fully and partially drawing) of undrawn polyester yarns should be emphasized, because of the improvement in uniformity that results. External heaters are an inevitable source of variability, and therefore non-uniformity, end-to-end, as well as along-end. The latter improvement also improves tensile properties and uniformity of shrinkage. Use of heaters also leads to "stop-marks" in the resulting fabrics, which can be avoided by cold-drawing. Uniformity is also affected by any lack of uniformity in the feed yarns, e.g., non-uniform interlace.

The tensiles are measured in the Example and shown in Tables I-III first on yarns AW, then ABO and also ADH, meaning, respectively, "As Warped", "After Boil-Off" and "After Dry Heat", to distinguish the state of the yarns at different stages of textile processing, it being understood that some of the values were measured on yarn taken from tubes, e.g., for comparison yarns, while others were taken from beams.

The importance of large crystals has already been mentioned hereinabove, and by Knox and Frankfort &

Knox, and their presence is shown by the density and crystal size, which should be as already mentioned. These parameters distinguish the feed yarns and the resulting drawn products from all conventional drawn yarns, from conventional POY and from spin-oriented yarns spun at low speeds, as described in those patents. Preferably, the drawn products are of density about 1.37 to about 1.415 g/cm<sup>3</sup>.

The relationship between crystal size (CS) and density ( $\rho$ ) is illustrated in FIG. 4, for both feed yarns and drawn yarns, whereas in FIG. 5, the relationship between RDDR and  $\sqrt{PYM}$  is illustrated.

The Relative Disperse Dye Rate, as defined and described by Knox, is significantly better than for conventional drawn polyester, and is preferably at least 0.09, for the drawn products, despite the fact that they have been drawn. The combination of this good dyeability (reduced from the corresponding feed yarns to an extent that depends on the drawing conditions and any heat setting) with tensile properties that are improved, especially the absence of any yield zone, as shown by the range of post yield modulus indicated above, distinguishes the novel drawn products from the prior art.

The K/S Dye Uptake values herein in Tables I, II and III were measured (as described by Frankfort & Knox, except that a McBeth spectrophotometer was used) on fabrics dyed with 4% on weight of fabric (OWF) of Teranil Yellow 2 GW in a bath buffered to a pH of 5.5, boiled for 25 minutes, whereas the fabrics for Table IV were dyed with 4% OWF of Blue GLF at 95° C. for 60 minutes.

The Jersey Warp Knit fabrics were dyed in a minijet, with 1.5% OWF Eastman Polyester Blue GLF at a pH buffered to 5.0-5.5 for 40 minutes under pressure at 260° F. so as to favor the fabrics that do not have easy dye-at-boil characteristics (Tables II/III). If the fabrics had been dyed at the boil, those in Table I would have been well and uniformly dyed, whereas those in Table II/III would not have dyed very well and would have been even less uniform than shown in Table II/III.  $\Delta Wt/$ Area % is a measure of area fabric shrinkage during this dyeing and subsequent heat-setting (dry at 300°-350° F. for 1 minute exposure with 5% overfeed).

The fabrics in Tables I, II and III were judged for dye uniformity and appearance as follows:

Fabric swatches (full width, i.e., approximately 20 inches wide and about 20-25 inches long) were laid on a large table covered with dull black plastic; the room lighting was diffuse fluorescent light. Four different attributes were judged:

(a) long streaks, i.e., those that persist throughout length of fabric sample and that are parallel to the selvage;

(b) short, hashy streaks, i.e., those that do not persist throughout the length of the fabric sample;

(c) dye mottle, i.e., spotty pattern of light and dark regions, the spots being one or a few millimeters in diameter;

(d) deep dye streaks, i.e., intensely colored parts of the fabric, the color intensity being higher than the average of the fabric sample;

The rating scale is:

5 = no defect visible, absolutely uniform;

4 = minor unevenness observed, acceptable for almost all end uses;

3 = unevenness noticeable, not usable for high quality goods, may be used for utility apparel, second grade clothes;

2 = unevenness highly noticeable, too uneven for any apparel;

1 = extremely uneven, disastrously defective.

Each fabric sample was paired against each of the others and thus rated, such that the resulting ratings scaled the fabrics in this series. The fabrics and their ratings were given to laboratory colleagues for critique and found to be consistent and acceptable.

The Mullen Burst Test is a strength criterion for fabrics and was measured (lbs/in) according to ASTM 231-46. The Burst Strength is obtained by dividing the Mullen Burst by the Area Weight (oz/sq yd). Fabrics from drawn filament yarns according to the invention preferably have Burst Strengths (ABO) in the approximate range 15-35 (lbs/in)/(oz/sq yd) and also greater than about the value defined by the following relationship:

Burst Strength (ABO) > 31[1 -  $E_B$ (ABO)/100], where  $E_B$ (ABO) ≈ 100[( $E_B$  +  $S_1$ )/(100 -  $S_1$ )], and where  $S_1$  and  $E_B$  are the boil-off shrinkage and elongation-to-break, respectively, as already mentioned. Burst strength (ABO) is preferably expressed in terms of  $S_1$  and  $E_B$  using the above expression for  $E_B$ (ABO) to give the following relationship:

$$\text{Burst strength (ABO)} > 31[1 - (E_B + S_1)/(100 - S_1)].$$

FIG. 6 illustrates the Burst Strength plotted against  $E_B$  (ABO) for drawn yarns (AW) of  $E_B$  about 20-90% and  $S_1$  < 10%, with preferred drawn yarns (AW) of  $E_B$  about 20-60% and  $S_1$  < 6%.

The intrinsic viscosity [ $\eta$ ] is generally in the approximate range 0.56-0.68 for textile yarns.

Preferred birefringence values for the feed yarns are in the approximate range 0.05-0.12, especially 0.05-0.09, and are correspondingly higher for the drawn products, namely 0.07-0.16. Birefringence values are very difficult to measure unless the yarns are of round cross section, and there is an increasing tendency for customers to prefer various non-round cross sections, because of their aesthetics.

Draw-warping may be carried out according to the directions of the manufacturers of the various commercial machines. The warp draw ratio (DR) will generally be given by:

$$DR \leq \frac{100 + E_B}{100} \div (RDR)_D$$

where  $E_B$  is the elongation of the feed yarns and  $(RDR)_D$  is the residual draw ratio of the resulting warp-drawn yarns, and, using  $E'_B$ , the elongation of such warp-drawn yarns, instead of the feed yarns, may be given by:

$$(RDR)_D = \frac{100 + E_B}{100}$$

This  $(RDR)_D$  will generally be more than about 1.1×, and especially more than about 1.2×, i.e. to give corresponding  $E'_B$  of more than 10%, and especially 20% or more, but this is largely a matter of customer preference.

Relative denier spread and Uster data as reported in Tables VII-XII are the ratios of the % coefficient of variations of results measured on warp-drawn yarns and corresponding feed yarns. The denier spread and Uster

data are measured on a Model C-II Uster evenness tester, manufactured by Zwellweger-Uster Corporation. The denier spread data, which relate to long-term variations in yarn uniformity, are based on samples measured under the following conditions:

Yarn speed—200 meters/minute  
Machine sensitivity—12.5 (inert setting)  
Evaluation time—2.5 minutes  
Chart speed—10 cm./minute

Uster data, which relate to short-term variations in yarn uniformity, are measured at:

Yarn speed—25 meters/minute  
Machine setting—normal  
Evaluation time—1 minute  
Chart speed—100 cm./minute

Draw tension variation along the length of a continuous filament yarn is a measure of the along-end orientation uniformity and relates to dye uniformity. Yarns having a high draw tension variation give nonuniform, streaky dyed fabrics. Draw tension is measured with a Extensotron® Model 4000 transducer equipped with a 1000 gram head which is calibrated at 200 grams, and the yarns are drawn at the RDR's specified while passing at an output speed of 25 meters/minute through a 100 cm. long tube heated to the temperature that is specified. The average draw tension is determined from 500 measurements, and the percent coefficient of variation is calculated and reported.

The parent invention lends itself to many variations, some of which are now described briefly:

1. (A) -Co-draw nylon POY (which can be cold drawn and partially drawn too) and the preferred feed yarns described herein, to provide a nylon/polyester mixed yarn warp.

(B) -Use heat-setting to reduce level of shrinkage and differential shrinkage of yarns if desired for any end-use.

2. Co-draw preferred feed yarns of different cross sections/deniers for a patterned warp, all at same shrinkage level. Use heat-setting to reduce level of shrinkage and differential shrinkage of yarns if desired for any end-use.

3. Co-draw split warp sheets, some cold and others with heat, to give a mixed shrinkage pattern warp.

4. Variable along-end heating would give varying shrinkage, and so give a patterned warp.

5. Use preferred feed yarns of different heat setting capability.

6. Use draw-warping to reduce denier and obtain unusually low denier warps.

7 Co-draw more than one beam, some of which have been alkali treated and then break the alkali-treated ends to give spun-like effect.

8. Hot draw in a bath containing dyestuffs, UV-screener, or other additives to take advantage of high dye rate of the preferred feed yarns.

9. Cold draw with or without post-heat setting single ends of preferred feed yarns, for use as filling yarns. This could be performed on the loom itself.

10. Edge-crimp while cold-drawing preferred feed yarns. The resulting 8-10% shrinkage plus subsequent 1-2% elongation would give crimped yarns in fabric.

11. Use additives to increase light fastness of the preferred feed yarns.

From the foregoing, it will be clear that there are many ways to take advantage of the benefits of the preferred feed yarns in various drawing processes as described herein. The main advantages of these feed yarns over conventional POY can be summarized as:

1. Reduced sensitivity to heat means the eventual fabrics will be more uniform, and there is less potential for stop-marks.

2. By using the ability for cold-drawing, significantly improved uniformity can be obtained, with a useful combination/balance of tensile and shrinkage properties. This can be used to improve the tensiles (yield zone) with only slight loss of the improved dyeability of the feed yarn, so that it can be used, e.g., as a filling yarn for weaving, or for drawing and airjet texturing or for drawing and crimping for staple.

3. The process can involve less trimer production and fuming of the finish, which can lead to other advantages, for instance the feed yarn manufacturer can apply a finish that will persist and remain satisfactory beyond the draw-warping operation, i.e., reduce or avoid the need to apply further finish for weaving or knitting.

4. The resulting drawn products have generally higher rate of alkali weight reduction than conventionally drawn POY and fully drawn yarns.

5. The flexibility for the draw-warper to custom-tailor his desired combination of tensiles, shrinkage, dyeability and denier over a large range of draw-ratios while maintaining uniformity may be most prized advantage of many fabric designers.

6. The resulting drawn products have lower modulus than conventional drawn polyester, and so have generally better aesthetics.

7. Any type of draw-warping machine can be used, or even a tenter frame or slasher unit, for example, modified to incorporate warp beaming.

Indeed, further modifications will be apparent, especially as these and other technologies advance. For instance, any type of draw winding machine may be used. Also, as regards variation 9, for example, the yarns may have any end uses that have been or could be supplied by fully oriented yarns, including west knitting yarns, and supply yarns for twisting and draw winding.

## EXAMPLES

In the following Example, 6 separate draw-warping operations are carried out first according to the invention of the parent application. Table I shows for these operations (designated I-1 through I-6) yarn characteristics, warping conditions and fabric characteristics, and includes appropriate corresponding details for yarns that were not processed according to the invention (designated IA, IB and IC) so that their characteristics may be compared with yarns (I-1 through I-6) warp-drawn according to that invention.

Following Table I, details are given in Comparison Tables II and III for warp-drawing other control yarns, i.e. these warp-drawing processes were also for purposes of comparison only.

Following Tables II and III, another series of 8 draw-warping operations were carried out according to the invention of the parent application, with details given in Table IV, and designated as IV-2 through IV-9. IV-1 is merely the feed yarn used for these draw-warping operations.

Following Table IV, several important characteristics of the feed yarns used for draw-warping are compared side-by-side for convenience in Tables V and VI. V-3 was a feed yarn used to carry out the draw warping processes according to the invention of the parent application, as shown in Tables I and IV, whereas V-1 is the feed yarn used in Comparison Table II and V-2 is the feed yarn used in Comparison Table III. Similarly VI-3

was used according to that invention, whereas VI-1 and VI-2 were used for comparison experiments. The results are shown in the later Tables.

As disclosed in the Example and hereinbefore, the drawing can be carried out under various conditions. Cold-drawing is the term used when no external heat is applied; but, as is well known, exothermic heat of drawing and the friction of the running threadline will generally and inevitably heat any snubbing pin unless specific means are used to avoid or prevent this. Cold-drawing will generally somewhat raise the shrinkage of the resulting drawn yarn; this may be tolerable, depending on the balance of properties desired, and may be desirable for certain end-uses. Hot-drawing, where the feed yarn is heated, or when a cold-drawn yarn is annealed after drawing, will enable the operator to produce drawn yarns of low shrinkage, similar to that of the feed yarn; this will also reduce the dyeability somewhat, but the resulting dyeability will still be significantly higher than that of conventional drawn polyester.

The parameters of the test feed yarns in the Example were within the preferred ranges specified hereinabove. The draw-warping processes were carried out on an apparatus provided by Karl Mayer Textilmaschinenfabrik GmbH, D-6053 Oberhausen, Germany, illustrated schematically in FIG. 1, with reference to the Karl Mayer machine, (other commercial machines have also been used successfully and have arrangements that are somewhat similar or analogous). A sheet of warps is drawn by feed rolls 1A and 1B from a creel (not shown) on the left and is eventually wound on a beam 8 on the right of FIG. 1. Feed rolls 1A are heatable, if desired, whereas feed rolls 1B are non-heatable. The warp sheet then passes up in contact with an inclined plate 2, that may, if desired, be heated so as to preheat the warps, before passing over a heatable pin 3, sometimes referred to as a snubbing pin, and then down in contact with another inclined plate 4, which may, if desired, be heated so as to set the drawn warps before passing to the set of draw rolls 5A and 5B, that are driven at a greater speed than the feed rolls, so as to provide the desired warp draw ratio, and wherein draw rolls 5A may be heated if desired, whereas draw rolls 5B are non-heatable. The warps may, after leaving the draw rolls 5A and 5B, bypass directly to the beam winder 8, as shown in one option in FIG. 1, or may, if desired, undergo relaxing by passing down in contact with another inclined plate 6, which may be heated to relax the warps as they pass to a set of relax rolls 7A and 7B, that are driven at a speed appropriately less than that of the draw rolls, so as to provide the desired overfeed, and, wherein relax rolls 5A may be heated, if desired, whereas relax rolls 5B are non-heatable, before passing to beam winder 8.

#### PARENT EXAMPLE

This first compares the results of six draw-warping processes according to the invention of the parent application (tests I-1 to I-6), using feed yarns of 108 denier, 50 filament (trilobal), that are spin-oriented with large crystals as described above, on the one hand, in contrast with two conventional drawn polyester yarns IA and IB and with a spun-oriented direct-use polyester yarn IC so to contrast the properties of these drawn yarns (tests I-1 through 6 and IA,B) and of the direct-use yarn IC and of fabrics made therefrom. Item IC is not a drawn yarn but a spun-oriented direct-use yarn that was also the feed yarn used to prepare yarns I-1 through I-6

(to show the effects of the draw-warping processes) and fabrics therefrom.

Tests 1 and 6 were essentially fully drawn to residual elongations of 25.4% and 30.7%, respectively, which correspond to residual draw ratios (RDR) of  $1.254\times$  and  $1.307\times$ , respectively. Yarns in Tests 2 through 5 were drawn at lesser draw ratios to residual elongations greater than 30%, corresponding to a residual draw ratio (RDR) greater than  $1.3\times$ . Yarns in Tests 4-6 were drawn cold (without externally-applied heat) wherein the heat of draw and friction increased the temperatures to about 70° C. All test yarns gave acceptable tensiles as indicated by an initial modulus (M) greater than 40 g/d, a tenacity at 7% elongation ( $T_7$ ) of 1 g/d or greater and an elongation to break ( $E_B$ ) less than 90% and especially less than 60%. The test yarns also maintained acceptable tensiles after boil-off shrinkage (ABO) and after dry heat shrinkage (ADH). The retention of tensiles after exposure to heat is attributed to a combination of densities ( $\rho$ ) greater than about 1.355 g/cm<sup>3</sup> (and especially greater than about 1.37 g/cm<sup>3</sup>) and very large crystals characterized by a wide-angle X-ray (WAXS) crystal size (CS) of at least 60 Angstroms and greater than about (250 $\mu$ -282.5) Angstroms. The thermal stability ( $S_2$ ) is characterized by the additional change in yarn length on heating to 350° F. (177° C.) of less than about 2% (the (1.6) figure indicating an increase in length of 1.6% for I-4) after initial boil-off shrinkage ( $S_1$ ) of less than about 10% and preferably less than about 6%, giving a net shrinkage ( $S_{12}=S_1+S_2$ ) of less than about 8% and preferably less than about 6%.

In contrast, commercially available fully drawn hard yarns (IA and IB) have much inferior thermal stability ( $S_2$ ) values of about 5% and net shrinkages ( $S_{12}$ ) of about 12%, because they have smaller crystals of crystal size (CS) of 56 Angstroms and 44 Angstroms, respectively. The fully drawn hard yarns (IA and IB) also show about a 50% reduction in their initial tensiles (e.g., modulus, M, and tenacity at 7% elongation,  $T_7$ ) after shrinkage (ABO) and (ADH).

The test yarns (I-1, 2, 3, 5 and 6) have similar thermal stability to the commercially available direct-use yarn (IC), but sustained tensiles, as characterized by a tenacity at 7% elongation ( $T_7$ ) of greater than about 1 g/d and a post yield modulus (PYM) before and after boil-off of at least 5 g/d.

The test yarns (I-1 through 6) are further characterized by an improved dyeability as indicated by a Relative Disperse Dye Rate (RDDR) of at least 0.075 and preferably of at least 0.09 and greater than (0.165-0.025  $\sqrt{PYM}$ , ABO). The test yarns have RDDR values 1.5 $\times$  to 3 $\times$  fully drawn hard yarns and depending on warp-draw process conditions, RDDR values nearly comparable to the commercially available direct-use yarn IC. Drawing the test yarns without added heat (i.e., cold, except for internal heat of draw) enhances dyeability, whereas external heat in general lowers dyeability.

The test yarns (I-1 through 6) were knit into Jersey warp knit fabrics and dyed under commercial conditions—i.e., similar to those used for fabrics made with fully drawn hard yarns—but with a critical disperse dye (Blue GLF) to enhance non-uniformity. All test yarns give very uniform fabrics, comparable to commercially available fully drawn hard yarns (IA) and direct-use yarns (IC). This was unexpected since test yarns (I-2 through 5) were drawn to residual elongations greater

than 30% and test yarns (I-4 through 6) were drawn cold.

The retention of uniformity is attributable to this unique and surprising capability of these test yarns to be partially drawn (hot or cold) to such residual elongations as are greater than 30%, and even greater than 40%, while maintaining uniform along-end denier and shrinkage properties. This unique capability of uniform drawing is believed to be due to a combination of an initial yield stress ( $\sigma_y$ ) of at least about 0.8 g/d and preferably 0.9 g/d which approximately corresponds to a tenacity at 7% ( $T_7$ ) of at least about 0.7 g/d and preferably 0.8 g/d and a yield zone ( $E'' - E'$ ) less than about 15% and preferably less than about 10% and a crystal structure characterized by large crystals of crystal size (CS) of at least 55 Angstroms and greater than about (250  $\mu$ -282.5) Angstroms for density ( $\rho$ ) values 1.35-1.39 g/cm<sup>3</sup>. The unique crystal structure is believed to permit the yarns to draw in a uniform manner, similar to nylon, without neck-drawing which would give rise to along-end denier and shrinkage non-uniformity.

The test yarn fabrics (I-1 through 6) also show improved thermal stability as characterized by  $\Delta Wt/area$  (%) values less than the commercially available fully drawn hard yarn (IA). The test yarn fabrics (I-1 through 6) also had acceptable Burst Strengths (ABO) of at least 15[(lbs.yd<sup>2</sup>)/(oz.in)] and greater than about 31[1-( $E_B + S_1$ )/(100-S<sub>1</sub>)] where  $E_B$  and  $S_1$  are measured on the yarns (AW).

An important advantage when cold draw-warping was performed, was the absence of stop-marks on the resulting fabrics.

Although the draw-warping machine used in this Example was manufactured by Karl Mayer, the process has also been demonstrated with other machines, including draw-warping machines manufactured by Liba-Barmag and by Val Lesina, and slashers manufactured by Tsudakoma Corp.

The following abbreviations have been used in the Tables.

PY=Post Yield

RT=Room Temperature;

RND=Round;

TRI=Trilobal

ABO=After Boil-Off;

ADH=After Dry Heat;

AW=As Warped

OFF=Not heated; measured at approx. 70° C. due to heat of friction and draw

EWDR=WDR × [(100-% over feed)/100]  
 $\Delta Wt./Area$  (%)=[1-Area Wt. (finished)/Area Wt. (greige)]100

Burst Strength=Mullen Burst/Area Wt.

\* (Corrected for TiO<sub>2</sub> pigment)

In Comparison Tables II and III, commercially available partially oriented yarns (POY) such as are used as feed yarns for draw-texturing were selected as control yarns for feeding to same draw-warping machine. Control yarn II is a nominal 115-34 trilobal POY with 0.035% TiO<sub>2</sub> and 0.658 intrinsic viscosity and is characterized in detail hereinafter as V-1 in Table V. Control feed yarn III is a nominal 107-34 round POY with 0.30% TiO<sub>2</sub> and of 0.656 intrinsic viscosity and is characterized in detail hereinafter as V-2 in Table V. Control feed yarn V-1 was draw-warped to a residual elongation of about 24% using temperatures similar to test I-1 and 2, except the set plate was at 160° C. The draw-

warped yarn II-1 had poorer thermal stability than test yarns I-1 through 6, as characterized by an  $S_2$  value >2% and a net shrinkage ( $S_{12}$ ) greater than 8%. The dyeability of II-1 was significantly lower than the test yarns I-1 through 6 with an RDDR value of 0.062, or less than 0.075. The poorer dyeability is consistent with crystal size (CS) less than 60 Angstroms. Although the dyed Jersey warp knit fabrics had acceptable thermal stability and Burst Strength as indicated by  $\Delta Wt/area$  of 29.4% and a Burst Strength of 26.6 (lbs.yd<sup>2</sup>)/(oz.in), the dyed fabrics had poorer uniformity v. fabrics from test yarns (I-2 through 5), drawn to higher residual draw ratios.

The control feed yarn V-2 was draw-warped under identical conditions as the test yarn (V-3) except the draw ratio was increased because of the higher initial elongation-to-break ( $E_B$ ) versus the test yarn. The control draw-warped yarns III-1 and 6 were fully drawn; III-2 to 5 were partially drawn; and III-4 through 6 were drawn without heat added. Control yarn III-5 was nearly fully drawn to a residual elongation of about 30% and then relaxed 10% to a final residual elongation-to-break of about 43%.

The dyeability of all the draw-warped POY (control yarns II and III) were poorer than that of the test yarns (I), except for III-4 which was drawn cold and had an excessive net shrinkage of 18.6%. The poorer dyeability of the control yarns II and III is consistent with smaller crystals of crystal size (CS) less than about (250 $\mu$ -282.5) Angstroms.

The dyed warp knit Jersey fabrics (III-1 through 6) had poorer uniformity than the corresponding test yarn fabrics (I-1 through 6) supporting the observation that conventional POY cannot be partially drawn as uniformly as the test feed yarn used here wherein selected combinations of initial yield properties and unique crystal structure provides a feed yarn that can be drawn to any residual draw ratio (hot or cold) and give a uniform yarn with acceptable tensiles and better thermal stability and dyeability than conventional drawn polyester. This can be illustrated by comparing the along-end denier uster traces of the actual drawn yarns. This has been done for three sets of yarns in FIGS. 7, 8 and 9. Thus FIG. 7 compares such Uster traces for control yarn III-1 vs. test yarn I-1, while FIG. 8 compares control yarn III-2 vs test yarn I-2, and FIG. 9 compares control yarn III-4 vs. test yarn I-4. The better uniformity of each such test yarn is very evident from each Figure.

Referring to Table IV, yarn IV-1 is a round nominal 75-40 filament yarn which was treated under different drawing and overfeed conditions on a single-end basis (IV-2 through IV-9). Drawing and/or heat treatments increase the orientation (birefringence,  $\Delta n$ ) and density,  $\rho$ , of the test yarn IV-1. The initial tensiles as characterized by the initial modulus, M, and tenacity at 7% elongation ( $T_7$ ) were enhanced, except for the modulus values of yarns IV-2, IV-4 and IV-6 which were obtained under these conditions: draw temperatures of about 100° C., presence of water, and drawing conditions ranging from slight relaxation to slight draw. The yarns are characterized by low shrinkage of less than 6% and low shrinkage tension (ST) less than 0.15 g/d, except for yarns IV-8 and 9 drawn 1.10 $\times$ . All yarns had good dyeability similar to the feed yarn, except for yarns IV-7 and 9 drawn 1.05 $\times$  and 1.10 $\times$ , respectively, at 180° C., which have somewhat lower dyeability.

The improvements to the yarn mechanical properties by various heat treatments are further illustrated by comparison of the Load-Elongation curves of the yarns in Table IV. In FIG. 18, curves a, b and C represent yarns IV-3, IV-2 and IV-1, respectively, and are compared. In FIG. 19, curves a-d represent yarns IV-9, IV-7, IV-5, and IV-1 respectively, and are compared. In FIG. 20, curves a-d represent yarns IV-8, IV-6, IV-4, and IV-1, respectively, and are compared. In all cases, heat treatment, especially under tension or slight drawing, enhanced the mechanical properties of the test yarn IV-1 as a warp yarn for knitting and weaving.

The feed yarns are compared in Table V where V-1 and V-2 are commercially available POY used in the Example as the sources of control yarns II-1 and III-1 through 6, respectively, and V-3 is the test feed yarn used in the Example as the source of test yarns I-1 through 6, and is the direct-use yarn IC shown in Table I. The control feed yarns V-1 and V-2 differ significantly from the test feed yarn V-3 in that the yarns have lower yield points ( $\sigma'y$ ), longer yield zones ( $E''-E'$ ), and poorer thermal stability with boil-off shrinkages greater than 10%. The control feed yarns had densities less than  $1.35 \text{ g/cm}^3$  and very small crystals giving diffuse scattering by wide-angle X-ray (WAXS).

Additional feed yarns are compared in Table VI where yarns VI-1 and VI-2 are commercially available POY, similar to yarns V-1 and V-2 used in the Examples II and III, and are used as the sources of control yarns VII-1 through VII-6 and VIII-1 through VIII-6, X-1 through X-6 and XI-1 through XI-6,  $\times$ III-1 through XIII-8 and XIV-1 through XIV-8, respectively; and yarn VI-3 is the test feed yarn used as the source for test yarns IX-1 through IX-6,  $\times$ II-1 through XII-6, and XV-1 through XV-5, and is similar to the direct-use yarn IC shown in Table I. The control feed yarns VI-1 and VI-2 differ significantly (from the test feed yarn VI-3) in that they have lower yield points ( $\sigma'y$ ), longer yield zones ( $E''-E'$ ), and poor thermal stability with boil-off shrinkages greater than 10%. The control feed yarns had densities less than  $1.35 \text{ g/cm}^3$  and very small crystals giving diffuse scattering by wide-angle X-ray (WAXS). The load-Elongation curves are compared in FIGS. 10-12, and were obtained by drawing at  $19^\circ \text{ C.}/65\% \text{ RH}$  and 25 meters per minute using an along-end stress-stain analyzer manufactured entered by Micro Sensors Incorporated. The nonuniform neck yield region is very pronounced for the control yarns VI-1 and VI-2 in FIGS. 10 and 11, respectively, by the almost horizontal portions of the curves. The test yarn VI-3 does not exhibit neckdown, but uniform plastic flow behavior, as shown by its much more uniform along-end yield behavior in FIG. 12.

The commercially available POY VI-1 and VI-2 and the test yarn VI-3 were hot drawn at  $100^\circ \text{ C.}$  (Tables VII-IX, respectively) and cold drawn (Tables X-XII, respectively) over a wide range of draw ratios on an experimental single-end warp draw unit giving yarns of varying residual draw ratio (RDR). The control yarns VI-1 and VI-2, when partially drawn to RDR greater than about 1.3, had poor along end denier uniformity as shown by high values of relative Denier Spread, and relative Uster, and by short dark dye streaks (called mottle) in dyed knit tubing. The test yarn VI-3, however, could be partially drawn hot (Table IX) and cold (Table XII) to residual draw ratios (RDR) greater than about 1.3, and gave partially drawn yarns with acceptable along end denier uniformity and dyed knit tubing

essentially free of dye defects. The control yarns could only be drawn uniformly when drawn hot (Tables VI-IX) or cold (Tables X-XII) to residual draw ratios (RDR) of less than about 1.3. The test yarns, however, 5 still are preferred for drawing hot or cold to residual draw ratios less than about 1.3 as they gave improved along end uniformity (over the fully drawn control yarns) as indicated by lower values of relative along-end denier and Uster, and less visual dye defects (mottle) in the dyed knit tubing.

In FIGS. 13-15, along-end Uster traces are compared for the control yarns VII-2 and VIII-3 and test yarn IX-2, respectively, partially drawn hot to approximate residual draw ratios (RDR) of about  $1.5\times$ : that is to elongations in each of their respective "yield" regions. Only the test yarn had acceptable along-end Uster when partially drawn to within its yield region. The high relative Uster values of the control yarns (VII-2, for example) gave rise to pronounced dye mottle (DM) in dyed knit tubing while the test yarn IX-2 gave commercially acceptable uniformity with only a few faint dye streaks, as shown in FIGS. 16 and 17, respectively.

Another technique frequently used to define along end uniformity of the drawing process is the measurement of the coefficient variation (% CV) of the drawing tension (DT). In Tables XIII-XV, the control yarns VI-1 and VI-2 and the test yarn VI-3, respectively, were drawn over a wide temperature range from cold (the temperature in this case was defined here as  $19^\circ \text{ C.}$ ) 15 i.e. at room temperature, with no external heat added, to  $224^\circ \text{ C.}$ , and over a wide range of draw-ratios (1.1 to 1.9 $\times$ ) giving a corresponding wide range of residual draw ratios (RDR) of about 1.15 to  $2\times$ , depending on the particularly feed yarn's starting elongation. The control yarns VI-1 and VI-2 could not be partially drawn hot or cold to residual draw ratios (RDR) greater than about 1.3-1.4 as indicated by their high along end draw tension %CV values greater than 2%. The test yarn VI-3 could be uniformly partially drawn 30 hot and cold drawn over the entire draw ratio range tested as indicated by along end draw tension %CV values of less than 2%.

Warp beaming which includes a heat treatment to enhance yarn properties is incorporated, herein, as a form of "warp drawing" where the beaming can include relaxation, i.e., draw ratios of less than  $1.0\times$ , or restrained conditions, i.e., draw ratio of about  $1.0\times$ . Tenter Frames or Slasher units, for example, modified to incorporate warp beaming, are alternate forms of 35 warp treatment of which warp drawing is currently the most common. However, the test yarn of this invention makes the alternate warp treatments commercially viable routes to obtain enhanced warp yarn properties.

The feed yarns for use in this invention are highly 45 crystalline with excellent thermal stability and dyeability which characteristics may be essentially maintained after hot (or cold) drawing. These feed yarns are also capable of being drawn hot or cold uniformly to residual elongations greater than about 30%, which provides the flexibility of tailoring draw-warped yarns of given tensile, shrinkage, and dyeability for specific end-use requirements. Conventional POY cannot provide this flexibility in a single feed yarn.

#### MIXED SHRINKAGE EXAMPLES

Mixed shrinkage yarns have generally been formed previously by combining filaments of different shrinkage potential, wherein the differing shrinkage potentials

have, in part, been developed by differential drawing and/or by differential post heat treatment, and in part, by selecting different polymer compositions (e.g., relative viscosity and copolymers) with different propensities for crystallization during said drawing and/or heat treatments (such as disclosed in Reese, U.S. Pat. No. 3,444,681 and 3,998,042). Prior techniques disclosed for obtaining mixed shrinkage from a single polymer have been achieved by combining filaments of different shrinkage potential, developed typically by differential treatment of two filament bundles by heat (Maerov and McCord, U.S. Pat. No. 3,199,281), by asymmetric quenching (J.J. Kilian, U.S. Pat. No. 3,118,012), by applying spin finishes of different heat transfer characteristics (Reese, U.S. Pat. No. 4,153,660), by application of crystallizing solvents to one bundle, or by combining filament bundles of different filament deniers and/or cross-sectional shapes to provide differential surface-to-volume ratio (Jamieson and Reese, U.S. Pat. No. 2,980,492), and such filaments of differential shrinkage potential have been combined before or after drawing and heat treatment to provide fully drawn mixed shrinkage yarns with high shrinkage tensions (ST). Partial drawing of such conventional filaments (i.e., to residual elongations greater than about 30%) would have provided along-end "thick-thin" denier variability characteristic of intermittent neck-draw.

To provide uniform mixed shrinkage yarns, according to the present invention, however, filament bundles of differing shrinkage potential may be formed by high speed spinning, for example, of mixed-dpf filament yarns at 4 Km/min, wherein the high denier filaments have greater shrinkage than the low denier filaments. This is graphically represented in FIG. 21, wherein lines 1, 2 and 3 are plots of boil-off shrinkage ( $S_1$ ) against spin speed ( $V_S$ ) in Km/min, whereas line 4 is a plot of shrinkage tension (ST) against spin speed. Considering first line 1, this represents the fact that shrinkage ( $S_1$ ) increases with spin speed in the absence of any crystallization that is generally (in practice) induced by stresses during attenuation and quenching of the solidifying filaments. Line 3 represents a plot of boil-off shrinkage ( $S_1$ ) versus spin speed (in Km/min) for filaments ( $A_F$ ), such as POY, characterized by high shrinkage (e.g., as represented by feeder yarns of Piazza and Reese). Line 2 is a plot for filaments ( $B_F$ ), characterized by lower shrinkage (e.g., as disclosed by Knox). The fact, that the shrinkage ( $S_1$ ) of the ( $B_F$ ) filaments is lower is attributed to the greater amount of stress-induced crystallization. This difference enables one to combine spin-oriented filament bundles ( $A_F$ ) and ( $B_F$ ) and thereby provide mixed shrinkage (undrawn) yarns ( $AB_F$ ) from a single polymer source. These are referred to herein as Type C yarns (see Table XVII) Differential shrinkage may also be obtained by, but limited to, use of different polymer melt viscosities (e.g., via differential capillary shear and temperature of polymer feed streams), differential cooling (e.g., via differential convergence guide length, delay length, quench air rates/temperature, filament arrays), and are further illustrated in Table XVI.

Type C mixed shrinkage yarns (of undrawn filaments) are found to be unsuitable for tightly constructed knits and for most woven fabrics, because internal fabric yarn-to-yarn restraining frictional forces are not generally overcome by the low shrinkage tension of the yarns on heating. This limits the bulk developed, in practice in the fabrics, in contrast to what

might be expected from the differential shrinkage potential of yarn that is free from such restraints. Typically, such undrawn Type C yarns are characterized by (maximum) shrinkage tensions (ST) of about 0.1 g/d (herein also expressed as  $mg/d = 1000 \times g/d$ ). This may be seen from line 4 in FIG. 21, where the value of ST increases (with spin speed) through a value of 100 mg/d at a spin speed of about 5 Km/min, so is less than 100 mg/d at preferred spin speeds of about 4 Km/min. 5 However, post-bulking in fabrics typically requires shrinkage tensions (ST) significantly greater than even (0.15 g/d). So such Type C yarns may be "pre-bulked" 10 under relaxed conditions, prior to knitting and weaving; however, for a long time, it has been a more desirable 15 objective to provide mixed shrinkage yarns from a single polymer source that may also be usable in a large 20 range of fabric constructions without pre-bulking. The improved drawing process of the invention, described herein, provides uniform mixed shrinkage yarns with 25 differential shrinkage of at least about 5% and (maximum) shrinkage tensions (ST) at least about 0.15 g/d (i.e., at least about 150 mg/d). The present invention also provides a process for preparing uniform mixed shrinkage yarns of different deniers from the same feed 30 (herein after illustrated by yarn Types I-IV).

Example I-4 shows that cold drawing of low shrinkage undrawn textile yarns ( $B_F$ ), as described hereinbefore, increased the boil-off shrinkage ( $S_1$ ) from about 2-4% to about 8-10%, and increased shrinkage tension 35 (ST) to values greater than about 0.15 g/d, while maintaining thermal stability, as measured by an  $S_2$ -value less than about +1% and net shrinkage ( $S_{12}$ ) less than about 8%. Combining cold drawn filaments ( $B_D$ ) of the invention with the low shrinkage, undrawn filaments of same 40 said feed yarn ( $B_F$ ) can provide uniform mixed shrinkage filament yarns [herein denoted as Type I] with differential shrinkage of about 5% and maximum shrinkage tension (ST) greater than about 0.15 g/d. The undrawn filaments of the invention ( $B_F$ ) may be partially cold-drawn to provide for a broader range of 45 denier and tactile aesthetics (such as fabric drape), which is not possible with conventional drawing processes.

Alternatively, the undrawn low shrinkage feed yarns 50 of the invention ( $B_F$ ) may be cold drawn, as in preparing Type I yarns, but then said cold drawn filaments ( $B_D$ ) may be split into two drawn filament bundles, wherein one bundle is heat treated to reduce shrinkage ( $S_1$ ) and the second is not heat treated, and these filament bundles are combined to provide a drawn mixed 55 shrinkage filament yarn [herein denoted as type II], wherein the differential is about 5% and the shrinkage tension (ST) is greater than about 0.15 g/d. Both components of Type II yarn may be uniformly partially drawn to differing deniers without "thick-thin" sections to provide a broad range of aesthetics. A variation of Type II is to hot draw, with or without post heat treatment, one of the undrawn filament yarns ( $B_F$ ) to reduce 60 said shrinkage, and combine with the high shrinkage cold drawn filament yarns ( $B_D$ ) to provide for mixed-shrinkage filament yarns [herein denoted as Types III and IV, respectively] with greater differential shrinkage and lower shrinkage surface filaments than Types I and II mixed shrinkage yarns.

The drawing process of the invention may be used to 65 improve the properties of the mixed shrinkage undrawn filament yarns ( $AB_F$ ), described herein before, denoted as Type C yarns and illustrated in Table XVI, by pro-

viding said mixed shrinkage yarns with shrinkage tensions (ST) of at least about 0.15 g/d, wherein the low shrinkage drawn filaments ( $B_D$ ) are those previously described hereinbefore, and the high shrinkage drawn filaments ( $A_D$ ) are representative of drawn filaments of conventional POY (such as those described by Piazza and Reese). A mixed shrinkage yarn ( $AB_F$ ) comprised of undrawn filaments ( $A_F$ ) and ( $B_F$ ) is typically characterized by shrinkage tensions (ST) less than about 0.15 g/d. Cold drawing said mixed shrinkage undrawn yarn ( $AB_F$ ) without any post heat treatment provides for a mixed shrinkage drawn filament yarn [herein denoted as Type V] with a shrinkage tension (ST) greater than about 0.15 g/d, making said mixed shrinkage yarns suitable for post-bulk development in most fabric constructions (e.g., wovens).

Alternatively, the same undrawn filaments ( $A_F$ ) and ( $B_F$ ) of the mixed shrinkage undrawn yarn ( $AB_F$ ) may be supplied as separate undrawn feed yarns ( $A_F$ ) and ( $B_F$ ), wherein said feed yarns may be cold drawn and combined without any post heat treatment [Type VI], or the undrawn filament yarn ( $B_F$ ) may be cold-drawn followed by heat treatment [Type VII] or may be hot-drawn with post heat treatment [Type VIII] or without post heat treatment [Type IX] to further reduce shrinkage and increase overall differential filament shrinkage. In mixed-shrinkage yarns Type VI-IX the draw ratio of the A-filament yarns is generally selected to provide uniform drawn A-filaments with elongation-to-break ( $E_B$ ) less than about 30%. The draw-ratio of the B-filaments, however, may be varied over a wide range, to provide for different denier drawn filaments without "thick-thin" along-end denier variability which is characteristic of partially drawing, for example, the above high shrinkage filament feed yarns ( $A_F$ ).

Mixed shrinkage yarn Types V-IX, XIII, and XIV are characterized in that the shrinkages of drawn filaments ( $A_D$ ) are greater than that of drawn filaments ( $B_D$ ) (that is,  $S_A > S_B$ ). Mixed shrinkage yarns may be provided, wherein the shrinkage  $S_A$  is less than that of shrinkage  $S_B$ , by the cold drawing of the undrawn filaments  $B_F$  without any post heat treatment to provide uniform high shrinkage filaments which are then combined with drawn filaments ( $A_D$ ), wherein undrawn filaments  $A_F$  are drawn cold with post heat treatment, or drawn hot with or without post heat treatment to provide for mixed shrinkage drawn filament yarns (Types X-XII, respectively), wherein  $S_A < S_B$ . Mixed

shrinkage yarns may also be provided by co-mingling the undrawn filaments of the invention ( $B_F$ ) with or without post heat treatment, with cold drawn filaments ( $A$ ) (Types XIII and XIV, respectively).

In the above examples, the drawing and heat treatment may be carried out on single-ends to provide mixed shrinkage yarns on packages for circular knitting or for fill yarns for weaving, for example; or the drawing and heat treatment may be carried out on weftless warp sheets prior to warp knitting, weaving or winding onto beams. The bulk may be developed in fabric with conventional heat setting under relaxed conditions, or prior to knitting or weaving on single-end or on weftless warp sheets; and air-jet texturing of said pre-bulked or post-bulked yarns may be incorporated to provide unique textured bulky yarns and fabrics therefrom. To further enhance tactile aesthetics mixed dpf/cross-section filament yarns are preferred. The relative viscosity (LRV) of the polyester polymer is defined according to Broaddus U.S. Pat. No. 4,712,998.

Mixed shrinkage yarns Types X-XII provide low shrinkage surface filaments that are predominantly A-filaments, and high shrinkage core filaments that are predominantly B-filaments, whereas for yarns Types V-IX, XIII and XIV, the opposite is the case. Thus the process of the invention provides flexibility, in that, from the same source feed yarns (herein A and B), the surface and core filaments may be interchanged to provide for a wider range of visual and tactile aesthetics in the resulting yarns. For convenience, the yarn types C, and I-XIV are summarized in Table XVIII, wherein (B1/B2) denote 2 different yarn bundles of low shrinkage type B.

The shrinkage and shrinkage tension of the undrawn textile filament yarns used herein as filaments ( $B_F$ ), may be increased by rapid heating/cooling on the order of 100 degrees centigrade in less than one hundredth of a second while keeping said yarn under low tensions (i.e., about normal winding tensions). The heat may be provided by hot tubes, raising yarns to preferably about 100° C.-135° C., or by passing through a steam jet at 245° C. and 100 lb/in<sup>2</sup> pressure. The resultant yarns can be provided with (S<sub>1</sub>) and ST values greater than about 10% and 0.15 g/d and peak ST temperatures T(ST) less than about 100° C. High power filament yarns characterized by ST-values > 0.5 g/d and T(ST) > 100° C. are provided by increasing yarn temperatures to greater than about 150° C.

TABLE I

TABLE I-continued

|                                                         | YARN NO. |         |         |         |                      |         |         |        |         |
|---------------------------------------------------------|----------|---------|---------|---------|----------------------|---------|---------|--------|---------|
|                                                         | I-1      | I-2     | I-3     | I-4     | I-5                  | I-6     | IA      | IB     | IC      |
| <u>Shrinkages - AW, 5 mg/d</u>                          |          |         |         |         |                      |         |         |        |         |
| Boil-Off, S <sub>1</sub> (%)                            | 5.9      | 4.4     | 2.3     | 8.9     | 2.8                  | 1.7     | 6.7     | 7.0    | 3.4     |
| Thermal Stability, S <sub>2</sub> (%)                   | 1.2      | 0.7     | 1.2     | (1.6)   | 0.2                  | 1.1     | 5.1     | 5.3    | (0.3)   |
| Net, S <sub>12</sub> (%)                                | 7.1      | 5.1     | 3.5     | 7.3     | 3.0                  | 2.8     | 11.8    | 12.3   | 3.1     |
| Tension, ST (g/d)                                       | 0.42     | 0.24    | 0.22    | 0.17    | 0.03                 | 0.04    | 0.22    | 0.22   | 0.07    |
| <u>Tensiles - AW</u>                                    |          |         |         |         |                      |         |         |        |         |
| Modulus, M (g/d)                                        | 84.4     | 70.9    | 76.0    | 58.7    | 61.0                 | 70.4    | 117.6   | 99.9   | 49.5    |
| Ten. at 7%, T <sub>7</sub> , (g/d)                      | 2.2      | 1.7     | 1.8     | 1.4     | 1.3                  | 1.8     | 3.7     | 3.1    | 0.9     |
| Ten. at 20%, T <sub>20</sub> (g/d)                      | 3.6      | 2.5     | 2.8     | 2.1     | 2.4                  | 3.4     | 4.8     | 4.1    | 1.4     |
| PY Modulus, PYM (g/d)                                   | 15.1     | 9.1     | 11.0    | 7.9     | 11.5                 | 16.6    | 13.8    | 12.3   | 5.5     |
| Elongation, E <sub>B</sub> (%)                          | 25.4     | 42.8    | 40.0    | 48.4    | 45.2                 | 30.7    | 24.9    | 25.2   | 74.9    |
| Tenacity, T (g/d)                                       | 3.7      | 3.2     | 3.4     | 3.0     | 3.2                  | 3.7     | 5.1     | 4.3    | 2.7     |
| <u>Tensiles - ABO</u>                                   |          |         |         |         |                      |         |         |        |         |
| Modulus, M (g/d)                                        | 55.7     | 50.5    | 63.9    | 45.1    | 47.8                 | 54.6    | 54.6    | 52.1   | 54.8    |
| Ten. at 7%, T <sub>7</sub> , (g/d)                      | 1.7      | 1.3     | 1.6     | 1.0     | 1.2                  | 1.5     | 1.3     | 1.4    | 1.0     |
| Ten. at 20%, T <sub>20</sub> (g/d)                      | 3.1      | 2.1     | 2.5     | 1.7     | 2.3                  | 3.3     | 3.3     | 3.6    | 1.4     |
| PY Modulus, PYM (g/d)                                   | 14.6     | 8.7     | 9.9     | 7.5     | 11.4                 | 18.1    | 19.7    | 21.7   | 4.7     |
| Elongation, E <sub>B</sub> (%)                          | 31.2     | 48.0    | 43.2    | 56.4    | 44.2                 | 28.1    | 32.5    | 33.7   | 84.4    |
| Tenacity, T (g/d)                                       | 3.4      | 3.0     | 3.2     | 2.8     | 3.0                  | 3.4     | 3.6     | 3.8    | 2.6     |
| <u>Tensiles - ADH</u>                                   |          |         |         |         |                      |         |         |        |         |
| Modulus, M (g/d)                                        | 70.6     | 63.8    | 66.6    | 53.4    | 62.9                 | 62.0    | 51.7    | 53.6   | 43.9    |
| Ten. at 7%, T <sub>7</sub> , (g/d)                      | 1.5      | 1.3     | 1.4     | 1.1     | 1.4                  | 1.5     | 1.1     | 1.2    | 1.1     |
| Ten. at 20%, T <sub>20</sub> (g/d)                      | 3.2      | 2.3     | 2.4     | 1.9     | 2.4                  | 3.4     | 2.2     | 2.1    | 1.3     |
| PY Modulus, PYM (g/d)                                   | 17.2     | 10.5    | 10.6    | 8.5     | 10.6                 | 19.0    | 11.2    | 9.5    | 2.9     |
| Elongation, E <sub>B</sub> (%)                          | 34.2     | 50.1    | 47.3    | 56.0    | 43.8                 | 27.3    | 41.3    | 43.4   | 87.3    |
| Tenacity, T (g/d)                                       | 3.6      | 3.1     | 3.3     | 3.0     | 3.2                  | 3.5     | 3.6     | 4.1    | 2.8     |
| <u>Crystallinity - AW</u>                               |          |         |         |         |                      |         |         |        |         |
| Density, $\rho$ (g/cm <sup>3</sup> *)                   | 1.3810   | 1.3869  | 1.3998  | 1.3815  | 1.3864               | 1.3880  | 1.3758  | 1.3764 | 1.3624  |
| Crystal Size, CS (Å)                                    | 75       | 73      | 71      | 64      | 71                   | 72      | 56      | 44     | 66      |
| <u>Dyeability - AW</u>                                  |          |         |         |         |                      |         |         |        |         |
| Yarn                                                    | 0.093    | 0.123   | 0.121   | 0.154   | 0.129                | 0.098   | 0.062   | 0.045  | 0.164   |
| Rel. Disp. Dye Rate (RDDR)                              |          |         |         |         |                      |         |         |        |         |
| Fabric                                                  | 9.0      | 12.6    | 13.1    | 13.3    | 13.0                 | 9.9     | 6.5     | 8.7    | 16.2    |
| Dye Uptake (K/S)                                        |          |         |         |         |                      |         |         |        |         |
| <u>FABRICS</u>                                          |          |         |         |         |                      |         |         |        |         |
| Fabric Type                                             |          |         |         |         | → Jersey Warp Knit → |         |         |        |         |
| Course × Wale, greige                                   | 62 × 35  | 58 × 34 | 57 × 34 | 59 × 33 | 55 × 36              | 55 × 36 | 60 × 34 | —      | 60 × 34 |
| Course × Wale, finished                                 | 58 × 52  | 59 × 47 | 58 × 44 | 56 × 50 | 54 × 46              | 53 × 48 | 58 × 34 | —      | 60 × 34 |
| Area Wt. (oz/yd <sup>2</sup> ), greige                  | 3.88     | 4.12    | 4.18    | 4.09    | 4.27                 | 3.87    | 3.44    | —      | 4.58    |
| Area Wt. (oz/yd <sup>2</sup> ), finished                | 5.26     | 5.37    | 5.21    | 5.76    | 5.12                 | 4.82    | 4.98    | —      | 5.46    |
| ΔWt./Area (%)                                           | 35.6     | 30.3    | 24.6    | 40.8    | 19.9                 | 24.5    | 44.8    | —      | 19.2    |
| Mullen Burst (lbs/in)                                   | 135      | 111     | 103     | 101     | 101                  | 118     | 124     | —      | 84      |
|                                                         | 25.7     | 20.7    | 19.8    | 17.5    | 19.7                 | 24.5    | 24.9    | —      | 15.4    |
| Burst Strength (lb · yd <sup>2</sup> / oz · in)         |          |         |         |         |                      |         |         |        |         |
| <u>Dyed Fabric Rating</u><br>(1 = worst; 5 = no defect) |          |         |         |         |                      |         |         |        |         |
| Long streaks (LS)                                       | 5        | 4       | 4       | 5       | 4                    | 2       | 5       | —      | 5       |
| Short Streaks (SS)                                      | 3        | 3.5     | 4       | 4.5     | 4                    | 4       | 4       | —      | 3       |
| Dye Mottle (DM)                                         | 5        | 5       | 5       | 5       | 4                    | 4       | 5       | —      | 5       |
| Deep Dye Streaks (DDS)                                  | 5        | 5       | 5       | 5       | 5                    | 5       | 5       | —      | 5       |
| Average Rating (AR)                                     | 4.5      | 4.4     | 4.5     | 4.9     | 4.25                 | 3.75    | 4.75    | —      | 4.5     |

TABLES II and III

|                           | YARN NO. |        |        |        |        |        |        |
|---------------------------|----------|--------|--------|--------|--------|--------|--------|
|                           | II-1     | III-1  | III-2  | III-3  | III-4  | III-5  | III-6  |
| <u>Undrawn Denier</u>     |          |        |        |        |        |        |        |
| Warpden Denier            | 114.6    | 106.7  | 106.7  | 106.7  | 106.7  | 106    | 106.7  |
| Filaments - Shape         | 74.4     | 70.6   | 80.2   | 79.7   | 81.4   | 82.4   | 71.1   |
| TiO <sub>2</sub> , %      | 34 TRI   | 34 RND | 34 RND | 34 RND | 34 RND | 34 RND | 34 RND |
| Viscosity, [η]            | 0.035    | 0.30   | 0.30   | 0.30   | 0.30   | 0.30   | 0.30   |
| <u>WARPING CONDITIONS</u> |          |        |        |        |        |        |        |
| Draw Ratio, Speeds        |          |        |        |        |        |        |        |
| Warp Draw Ratio (WDR)     | 1.62     | 1.54   | 1.34   | 1.34   | 1.34   | 1.44   | 1.65   |
| Take-Up Speed (m/min)     | 500      | 500    | 500    | 500    | 500    | 500    | 500    |
| Relax/Overfeed (%)        | 0        | 0      | 0      | 0      | 0      | 10     | 10     |
| Effective WDR (EWDR)      | 1.62     | 1.54   | 1.34   | 1.34   | 1.34   | 1.30   | 1.49   |
| Temperatures (°C.)        |          |        |        |        |        |        |        |
| Feed Rolls                | 60       | 60     | 60     | 60     | 60     | RT     | RT     |
| Preheater Plate           | 86       | 86     | 86     | 86     | RT     | RT     | RT     |
| Draw Pin                  | 95       | 95     | 95     | 95     | OFF    | OFF    | OFF    |
| Set Plate                 | 160      | 170    | 170    | 195    | RT     | RT     | RT     |

TABLES II and III-continued

|                                                                                               | YARN NO. |         |         |                      |         |         |         |
|-----------------------------------------------------------------------------------------------|----------|---------|---------|----------------------|---------|---------|---------|
|                                                                                               | II-1     | III-1   | III-2   | III-3                | III-4   | III-5   | III-6   |
| <b>Relax Plate</b>                                                                            |          | RT      | RT      | RT                   | RT      | 195     | 195     |
| <b>YARNS</b>                                                                                  |          |         |         |                      |         |         |         |
| <b>Shrinkages - AW, 5 mg/d</b>                                                                |          |         |         |                      |         |         |         |
| Boil-Off, $S_1$ (%)                                                                           | 5.5      | 6.8     | 4.8     | 4.3                  | 25.8    | 1.6     | 2.1     |
| Thermal Stability, $S_2$ (%)                                                                  | 2.6      | 3.2     | 2.0     | 2.0                  | (7.2)   | 1.0     | 2.2     |
| Net, $S_{12}$ (%)                                                                             | 8.1      | 10.0    | 6.8     | 6.3                  | 18.6    | 2.6     | 4.3     |
| Tension, ST, (g/d)                                                                            | 0.22     | 0.41    | 0.22    | 0.22                 | 0.18    | 0.05    | 0.26    |
| <b>Tensiles - AW</b>                                                                          |          |         |         |                      |         |         |         |
| Modulus, M (g/d)                                                                              | 79.5     | 98.8    | 79.0    | 79.9                 | 60.0    | 70.5    | 81.4    |
| Ten. at 7%, $T_7$ (g/d)                                                                       | 2.7      | 3.4     | 2.0     | 2.1                  | 1.4     | 1.7     | 2.6     |
| Ten. at 20%, $T_{20}$ (g/d)                                                                   | 4.0      | 4.8     | 3.2     | 2.4                  | 2.2     | 3.2     | 4.8     |
| PY Modulus, PYM (g/d)                                                                         | 14.7     | 16.3    | 13.1    | 14.1                 | 8.8     | 15.5    | 22.9    |
| Elongation, $E_B$ (%)                                                                         | 24.4     | 24.2    | 42.3    | 38.2                 | 48.1    | 43.0    | 26.3    |
| Tenacity, T (g/d)                                                                             | 4.0      | 4.6     | 4.0     | 4.1                  | 3.5     | 4.1     | 4.8     |
| <b>Tensiles - ABO</b>                                                                         |          |         |         |                      |         |         |         |
| Modulus, M (g/d)                                                                              | 48.3     | 44.5    | 41.2    | 53.9                 | 37.7    | 60.8    | 50.2    |
| Ten. at 7%, $T_7$ (g/d)                                                                       | 1.5      | 1.7     | 1.3     | 1.5                  | 0.8     | 1.5     | 1.9     |
| Ten. at 20%, $T_{20}$ (g/d)                                                                   | 3.4      | 3.9     | 2.6     | 2.9                  | 1.1     | 3.0     | 4.5     |
| PY Modulus, PYM (g/d)                                                                         | 19.0     | 22.0    | 13.3    | 14.4                 | 2.8     | 15.3    | 25.9    |
| Elongation, $E_B$ (%)                                                                         | 30.7     | 28.8    | 44.3    | 40.0                 | 90.6    | 40.2    | 23.2    |
| Tenacity, T (g/d)                                                                             | 3.7      | 4.1     | 3.5     | 3.7                  | 2.6     | 3.7     | 4.3     |
| <b>Tensiles - ADH</b>                                                                         |          |         |         |                      |         |         |         |
| Modulus, M (g/d)                                                                              | 54.5     | 70.1    | 60.9    | 64.9                 | 12.5    | 66.7    | 63.5    |
| Ten. at 7%, $T_7$ (g/d)                                                                       | 1.4      | 1.6     | 1.3     | 1.4                  | 0.8     | 1.3     | 1.5     |
| Ten. at 20%, $T_{20}$ (g/d)                                                                   | 3.4      | 3.9     | 2.7     | 2.8                  | 1.0     | 2.8     | 4.3     |
| PY Modulus, PYM (g/d)                                                                         | 19.9     | 22.8    | 14.2    | 14.3                 | 1.8     | 15.1    | 27.3    |
| Elongation, $E_B$ (%)                                                                         | 31.6     | 32.2    | 47.1    | 43.0                 | 112.8   | 47.5    | 28.7    |
| Tenacity, T (g/d)                                                                             | 3.7      | 4.1     | 3.5     | 3.7                  | 2.6     | 3.7     | 4.3     |
| <b>Crystallinity - AW</b>                                                                     |          |         |         |                      |         |         |         |
| Density, $\rho$ (g/cm <sup>3</sup> )*                                                         | 1.3807   | 1.3824  | 1.3783  | 1.3838               | 1.3590  | 1.3940  | 1.3842  |
| Crystal Size, CS (Å)                                                                          | 52       | 58      | 53      | 61                   | Small   | 55      | 60      |
| <b>Dyeability - AW</b>                                                                        |          |         |         |                      |         |         |         |
| Yarn                                                                                          | 0.062    | 0.049   | 0.071   | 0.061                | 0.124   | 0.074   | 0.052   |
| Rel. Disp. Dye Rate (RDDR)                                                                    |          |         |         |                      |         |         |         |
| Fabric                                                                                        | 5.7      | 5.1     | 8.4     | 7.0                  | 9.3     | 8.0     | 5.6     |
| Dye Uptake (K/S)                                                                              |          |         |         |                      |         |         |         |
| <b>FABRICS</b>                                                                                |          |         |         |                      |         |         |         |
| Fabric Type                                                                                   |          |         |         | ← Jersey Warp Knit → |         |         |         |
| Course × Wale, greige                                                                         | 55 × 35  | 56 × 38 | 60 × 38 | 60 × 36              | 62 × 33 | 62 × 35 | 58 × 36 |
| Course × Wale, finished                                                                       | 56 × 47  | 56 × 50 | 56 × 50 | 56 × 50              | 67 × 58 | 56 × 50 | 56 × 44 |
| Area Wt. (oz/yd <sup>2</sup> ), greige                                                        | 3.40     | 3.41    | 3.85    | 3.84                 | 3.80    | 3.78    | 3.54    |
| Area Wt. (oz/yd <sup>2</sup> ), finished                                                      | 4.4      | 4.55    | 4.96    | 5.11                 | 6.57    | 5.03    | 4.05    |
| ΔWt./Area (%)                                                                                 | 29.4     | 33.4    | 28.8    | 33.1                 | 72.9    | 33.1    | 14.4    |
| Mullen Burst (lbs./in.)                                                                       | 117      | 123     | 113     | 110                  | 91      | 99      | 117     |
|                                                                                               | 26.6     | 27.0    | 22.8    | 21.5                 | 13.9    | 19.7    | 28.9    |
| Burst Strength $\left( \frac{\text{lb} \cdot \text{yd}^2}{\text{oz} \cdot \text{in}} \right)$ |          |         |         |                      |         |         |         |
| <b>Dyed Fabric Rating</b>                                                                     |          |         |         |                      |         |         |         |
| (1 = worst; 5 = no defect)                                                                    |          |         |         |                      |         |         |         |
| Long Streaks (LS)                                                                             | 4        | 4       | 3       | 2                    | 1       | 4       | 3       |
| Short Streaks (SS)                                                                            | 3        | 3       | 2       | 3                    | 5       | 4       | 3       |
| Dye Mottle (DM)                                                                               | 2        | 3       | 3       | 2                    | 5       | 2       | 3       |
| Deep Dye Streaks (DDS)                                                                        | 5        | 5       | 5       | 5                    | 1       | 5       | 5       |
| Average Rating (AR)                                                                           | 3.5      | 3.75    | 3.25    | 3                    | 3       | 3.75    | 3.5     |

TABLE IV

| YARN NO.                              | IV-1   | IV-2   | IV-3   | IV-4   | IV-5   | IV-6   | IV-7   | IV-8   | IV-9  |
|---------------------------------------|--------|--------|--------|--------|--------|--------|--------|--------|-------|
| Draw Ratio                            | —      | RELAX  | RELAX  | TAUT   | TAUT   | 1.05   | 1.05   | 1.10   | 1.10  |
| Draw Temperature (°C.)                | —      | 100    | 180    | 100    | 180    | 95     | 180    | 95     | 180   |
| Wet/Dry                               | —      | WET    | DRY    | WET    | DRY    | WET    | DRY    | WET    | DRY   |
| Density, $\rho$ (g/cm <sup>3</sup> )* | 1.3719 | 1.3877 | 1.3936 | 1.3862 | 1.3908 | 1.3756 | 1.3976 | 1.3801 | 1.397 |
| Birefringence ( $\Delta_n$ )          | 0.071  | 0.102  | 0.122  | 0.101  | 0.109  | 0.081  | 0.121  | 0.099  | 0.127 |
| Crystal Size, CS (Å)                  | 72     | 75     | 72     | 66     | 72     | 68     | 75     | —      | —     |
| Modulus, M (g/d)                      | 48.5   | 40.7   | 51.0   | 46.0   | 52.8   | 48.4   | 58.3   | 54.6   | 66.6  |
| Tenacity at 7%, $T_7$ (g/d)           | 0.9    | 1.0    | 1.2    | 1.1    | 1.2    | 1.1    | 1.3    | 1.3    | 1.3   |
| Elongation, $E_B$ (%)                 | 89.1   | 86.9   | 76.5   | 85.2   | 81.2   | 66.7   | 60.2   | 56.1   | 47.8  |
| Tenacity, T (g/d)                     | 3.0    | 2.9    | 2.9    | 2.9    | 3.0    | 2.9    | 3.0    | 3.0    | 3.0   |
| Shrinkage Tension, ST (g/d)           | 0.07   | 0.02   | 0.02   | 0.02   | 0.03   | 0.14   | 0.09   | 0.20   | 0.17  |
| Dye Uptake (K/S)                      | 17.7   | —      | —      | 15.6   | 16.3   | 16.7   | 12.2   | 16.8   | 10.7  |

TABLE V

| YARN NO.                                      | V-1    | V-2    | V-3    |
|-----------------------------------------------|--------|--------|--------|
| Undrawn Denier                                | 114.6  | 106.7  | 108.0  |
| Filaments - Shape                             | 34 TRI | 34 RND | 50 TRI |
| TiO <sub>2</sub> , %                          | 0.035  | 0.30   | 0.035  |
| Viscosity, [η]                                | 0.658  | 0.656  | 0.65   |
| Boil-Off Shrinkage, S <sub>1</sub> (%)        | 33.4   | 17.6   | 3.4    |
| Modulus, M (g/d)                              | 27.9   | 34.3   | 49.5   |
| Tenacity at 7% Elong., T <sub>7</sub> (g/d)   | 0.58   | 0.62   | 0.87   |
| Stress at 7% Elongation, σ <sub>7</sub> (g/d) | 0.62   | 0.66   | 0.93   |
| Yield Stress, σ <sub>y</sub> (g/d)            | 0.68   | 0.75   | 0.96   |
| Yield Zone, E'-E' (%)                         | 21.5   | 18.0   | 6.0    |
| Elongation to Break, E <sub>B</sub> (%)       | 118.4  | 95.8   | 74.9   |
| Uniform Partial Draw                          | No     | No     | Yes    |

 $\sigma = T_7 \times 1.07$ Stress,  $\sigma = (\text{Load (g)/initial denier}) \times (1 + \text{Elongation (\%)/100})$ E' = Elongation to yield point ( $\sigma'_y$ )E'' = Elongation to post yield point ( $\sigma''_y$ ), where ( $\sigma'_y = \sigma''_y$ )

TABLE VI

| Yarn No.                                      | VI-1   | VI-2   | VI-3   |
|-----------------------------------------------|--------|--------|--------|
| Undrawn Denier                                | 127.2  | 107.0  | 101.4  |
| Filaments - Shape                             | 34 RND | 34 RND | 50 TRI |
| TiO <sub>2</sub> , %                          | 0.30   | 0.30   | 0.035  |
| Boil-Off Shrinkage, S <sub>1</sub> (%)        | 54.8   | 11.1   | 3.2    |
| Modulus, M (g/d)                              | 22.0   | 25.1   | 36.6   |
| Ten. at 7% Elong., T <sub>7</sub> (g/d)       | 0.56   | 0.69   | 0.99   |
| Stress at 7% Elongation, σ <sub>7</sub> (g/d) | 0.60   | 0.74   | 1.06   |
| Yield Stress, σ <sub>y</sub> (g/d)            | 0.65   | 0.85   | 1.09   |
| Yield Zone, E'-E' (%)                         | 46     | 26     | 8      |
| Elong. at Break, E <sub>B</sub> (%)           | 136.2  | 120.7  | 73.3   |
| Uniform Partial Draw                          | NO     | NO     | YES    |

Yarns VI-1 thru VI-3 had a nominal Viscosity [η] of 0.65.

 $\sigma = T_7 \times 1.07$ Stress,  $\sigma = (\text{Load (g)/initial denier}) \times (1 + \text{Elong. (\%)/100})$ E' = Elongation to yield point ( $\sigma'_y$ )E'' = Elongation to post yield point ( $\sigma''_y$ ), where ( $\sigma'_y = \sigma''_y$ )

TABLES VII-IX

| Yarn No.                                | VI-1  | VII-1 | VII-2 | VII-3 | VII-4 | VII-5 | VII-6 | VI-2  | VIII-1 | VIII-2 |
|-----------------------------------------|-------|-------|-------|-------|-------|-------|-------|-------|--------|--------|
| Warp Draw Ratio, WDR                    | 1.00  | 1.39  | 1.48  | 1.57  | 1.69  | 1.82  | 1.97  | 1.00  | 1.22   | 1.30   |
| Residual Draw Ratio, RDR                | 2.36  | 1.59  | 1.51  | 1.41  | 1.35  | 1.21  | 1.12  | 2.21  | 1.72   | 1.63   |
| Elongation-to-Break, E <sub>B</sub> (%) | 136.2 | 58.9  | 51.1  | 40.8  | 34.5  | 21.2  | 12.3  | 120.7 | 71.7   | 62.6   |
| Rel. Denier Spread, WD/Feed             | 1.00  | 3.03  | 2.05  | 1.27  | 1.19  | 1.29  | 1.42  | 1.00  | 2.52   | 1.89   |
| Rel. Uster, WD/Feed                     | 1.00  | 7.58  | 5.12  | 2.33  | 1.58  | 2.69  | 1.79  | 1.00  | 5.67   | 4.03   |
| Dyed Fabric Ratings (DM)                | —     | 1     | 1     | 3     | 3     | 4     | 5     | —     | 1      | 1      |

  

| Yarn No.                                | VIII-3 | VIII-4 | VIII-5 | VIII-6 | VI-3 | IX-1 | IX-2 | IX-3 | IX-4 | IX-5 | IX-6 |
|-----------------------------------------|--------|--------|--------|--------|------|------|------|------|------|------|------|
| Warp Draw Ratio, WDR                    | 1.39   | 1.49   | 1.60   | 1.73   | 1.00 | 1.05 | 1.12 | 1.19 | 1.28 | 1.38 | 1.49 |
| Residual Draw Ratio, RDR                | 1.51   | 1.41   | 1.30   | 1.21   | 1.73 | 1.63 | 1.53 | 1.44 | 1.35 | 1.24 | 1.13 |
| Elongation-to-Break, E <sub>B</sub> (%) | 51.4   | 40.8   | 29.9   | 21.4   | 73.3 | 63.5 | 52.9 | 43.9 | 35.1 | 24.4 | 12.5 |
| Rel. Denier Spread, WD/Feed             | 0.98   | 0.81   | 1.00   | 0.88   | 1.0  | 0.79 | 0.67 | 0.47 | 0.72 | 0.61 | 0.94 |
| Rel. Uster, WD/Feed                     | 1.73   | 0.85   | 1.08   | 1.37   | 1.0  | 0.92 | 0.96 | 0.60 | 0.51 | 0.45 | 0.41 |
| Dyed Fabric Ratings (DM)                | 2      | 3      | 4      | 5      | —    | 4    | 4    | 4    | 5    | 5    | 5    |

WARP DRAW SPEED, METERS/MINUTE 600

PRE-HEATER PLATE TEMP., C. 90

DRAW PIN TEMP., C. 100

SET PLATE TEMP., C. 140

POST SET PLATE ROLL TEMP., C. 55

RELAXATION, % 0

TABLES X-XII

| Yarn No.                                | XI-1  | X-1  | X-2  | X-3  | X-4  | X-5  | X-6  | VI-2  | XI-1 | XI-2 | XI-3 | XI-4 |
|-----------------------------------------|-------|------|------|------|------|------|------|-------|------|------|------|------|
| Warp Draw Ratio, WDR                    | 1.00  | 1.39 | 1.48 | 1.57 | 1.69 | 1.82 | 1.97 | 1.00  | 1.22 | 1.30 | 1.39 | 1.49 |
| Residual Draw Ratio, RDR                | 2.36  | 1.56 | 1.52 | 1.44 | 1.31 | 1.22 | 1.14 | 2.21  | 1.69 | 1.60 | 1.48 | 1.37 |
| Elongation-to-Break, E <sub>B</sub> (%) | 136.2 | 55.5 | 51.6 | 43.9 | 30.8 | 21.7 | 14.0 | 120.1 | 69.2 | 60.1 | 47.6 | 36.8 |
| Rel. Denier Spread, WD/Feed             | 1.00  | 8.89 | 8.13 | 1.12 | 0.86 | 0.92 | 1.29 | 1.00  | 6.28 | 4.94 | 0.91 | 0.84 |
| Rel. Uster, WD/Feed                     | 1.00  | 8.57 | 5.40 | 1.26 | 1.05 | 1.12 | 1.64 | 1.00  | 4.30 | 3.00 | 0.82 | 0.75 |
| Dyed Fabric Ratings (DM)                | —     | 1    | 1    | 1    | 3    | 4    | 4    | —     | 1    | 1    | 1    | 2    |

  

| Yarn No.                                | XI-5 | XI-6 | VI-3 | XII-1 | XII-2 | XII-3 | XII-4 | XII-5 | XII-6 |
|-----------------------------------------|------|------|------|-------|-------|-------|-------|-------|-------|
| Warp Draw Ratio, WDR                    | 1.60 | 1.73 | 1.00 | 1.05  | 1.12  | 1.19  | 1.28  | 1.38  | 1.49  |
| Residual Draw Ratio, RDR                | 1.28 | 1.17 | 1.73 | 1.65  | 1.52  | 1.45  | 1.33  | 1.23  | 1.13  |
| Elongation-to-Break, E <sub>B</sub> (%) | 27.9 | 17.5 | 73.3 | 65.1  | 52.1  | 45.2  | 32.9  | 23.2  | 13.0  |
| Rel. Denier Spread, WD/Feed             | 0.69 | 0.83 | 1.0  | 0.96  | 1.14  | 0.83  | 1.27  | 0.86  | 0.93  |
| Rel. Uster, WD/Feed                     | 0.67 | 0.75 | 1.0  | 0.54  | 0.64  | 0.52  | 0.60  | 0.53  | 0.50  |
| Dyed Fabric Ratings (DM)                | 3    | 4    | —    | 4     | 4     | 4     | 5     | 5     | 5     |

WARP DRAW SPEED, METERS/MINUTE 600

PRE-HEATER PLATE TEMP., C. RT

DRAW PIN TEMP., C. RT

SET PLATE TEMP., C. 180

POST SET PLATE ROLL TEMP., C. RT

RELAXATION, % 0%

TABLES XIII-XV

| DRAW RATIO, YDR           | 1.1    | 1.2    | 1.3    | 1.4    | 1.5    | 1.6    | 1.7    | 1.8    | 1.9  |
|---------------------------|--------|--------|--------|--------|--------|--------|--------|--------|------|
| <u>Feed Yarn No. VI-1</u> |        |        |        |        |        |        |        |        |      |
| Drawn Yarn No.            | XIII-1 | XIII-2 | XIII-3 | XIII-4 | XIII-5 | XIII-6 | XIII-7 | XIII-8 |      |
| Residual Draw Ratio, RDR  | —      | 1.89   | 1.75   | 1.62   | 1.51   | 1.42   | 1.34   | 1.26   | 1.19 |
| <u>Draw Tension, % CV</u> |        |        |        |        |        |        |        |        |      |
| (Draw Temp., C.) - 19 C.  | —      | 2.8    | 2.1    | 3.1    | 4.2    | 6.7    | 2.9    | 3.8    | 4.2  |
| (Draw Temp., C.) - 79 C.  | —      | 4.8    | 4.3    | 3.2    | 4.2    | 4.6    | 3.4    | 2.1    | 4.5  |
| (Draw Temp., C.) - 100 C. | —      | 5.1    | 4.2    | 4.0    | 4.4    | 4.7    | 3.7    | 2.0    | 2.2  |
| (Draw Temp., C.) - 122 C. | —      | 4.3    | 4.8    | 5.2    | 4.9    | 4.0    | 2.6    | 1.7    | 2.3  |
| (Draw Temp., C.) - 174 C. | —      | 4.1    | 3.2    | 5.3    | 4.6    | 4.4    | 3.7    | 3.6    | 2.1  |

TABLES XIII-XV-continued

| DRAW RATIO, YDR           | 1.1   | 1.2   | 1.3   | 1.4   | 1.5   | 1.6   | 1.7   | 1.8   | 1.9 |
|---------------------------|-------|-------|-------|-------|-------|-------|-------|-------|-----|
| (Draw Temp., C.) - 224 C. | —     | 5.1   | 4.8   | 3.8   | 4.9   | 4.3   | 3.9   | 3.2   | 2.3 |
| Feed Yarn No. VI-2        |       |       |       |       |       |       |       |       |     |
| Drawn Yarn No.            | XIV-1 | XIV-2 | XIV-3 | XIV-4 | XIV-5 | XIV-6 | XIV-7 | XIV-8 |     |
| Residual Draw Ratio, RDR  | 2.01  | 1.85  | 1.70  | 1.58  | 1.47  | 1.38  | 1.30  | 1.23  |     |
| Draw Tension, % CV        |       |       |       |       |       |       |       |       |     |
| (Draw Temp., C.) - 19 C.  | 2.5   | 1.9   | 2.5   | 3.4   | 3.0   | 2.9   | 3.1   | 3.6   |     |
| (Draw Temp., C.) - 79 C.  | 3.2   | 3.6   | 3.2   | 2.7   | 2.0   | 1.5   | 1.4   | 1.8   |     |
| (Draw Temp., C.) - 100 C. | 2.7   | 3.4   | 3.8   | 2.1   | 2.1   | 1.4   | 1.0   | 1.5   |     |
| (Draw Temp., C.) - 122 C. | 3.1   | 3.0   | 3.5   | 2.5   | 2.1   | 1.8   | 1.2   | —     |     |
| (Draw Temp., C.) - 174 C. | 4.5   | 5.9   | 3.1   | 3.1   | 2.7   | 2.3   | 2.0   | —     |     |
| (Draw Temp., C.) - 224 C. | 4.0   | 4.5   | 4.1   | 3.1   | 2.5   | 2.0   | 3.4   | —     |     |
| Feed Yarn No. VI-3        |       |       |       |       |       |       |       |       |     |
| Drawn Yarn No.            | XV-1  | XV-2  | XV-3  | XV-4  | XV-5  |       |       |       |     |
| Residual Draw Ratio, RDR  | 1.57  | 1.44  | 1.33  | 1.24  | 1.15  |       |       |       |     |
| Draw Tension, % CV        |       |       |       |       |       |       |       |       |     |
| (Draw Temp., C.) - 19 C.  | 1.9   | 1.2   | 1.5   | 1.7   | 1.7   |       |       |       |     |
| (Draw Temp., C.) - 79 C.  | 3.2   | 1.8   | 0.9   | 0.8   | 0.9   |       |       |       |     |
| (Draw Temp., C.) - 100 C. | 2.3   | 1.6   | 1.2   | 1.0   | 0.9   |       |       |       |     |
| (Draw Temp., C.) - 122 C. | 2.0   | 1.8   | 1.3   | 1.1   | 0.9   |       |       |       |     |
| (Draw Temp., C.) - 174 C. | 2.6   | 2.1   | 1.4   | 1.1   | 0.9   |       |       |       |     |
| (Draw Temp., C.) - 224 C. | 3.7   | 2.4   | 1.6   | 1.4   | 1.0   |       |       |       |     |

MODEL 4000 EXTENSOTRON (TM) - MICRO SENSORS, INC. (New Englander Industrial Park, Holliston, Mass. 01746)

DRAW SPEED 25 METERS/MINUTE

DRAW ZONE 1 METER NONCONTACT HOT TUBE

SAMPLE LENGTH 50 METERS

TENSIONOMETER 1000 GRAM HEAD CALIBRATED TO 200 GRAMS

% CV DRAW TENSION 500 DATA POINTS

RESIDUAL DRAW RATIO, RDR = [1 + ELONGATION (%)/100%] feed / MACHINE DRAW RATIO

TABLE XVI

| EX. XVI-                   | 1       | 2       | 3       | 4       | 5       | 6       | 7      | 8       |
|----------------------------|---------|---------|---------|---------|---------|---------|--------|---------|
| SPIN SPEED, YPM            | 4500    | 4500    | 4000    | 4000    | 5000    | 5000    | 4500   | 4500    |
| SPIN SPEED, MPM            | 4115    | 4115    | 3658    | 3658    | 4572    | 4572    | 4115   | 4115    |
| [n]                        | 0.65    | 0.65    | 0.73    | 0.73    | 0.59    | 0.59    | 0.65   | 0.65    |
| T <sub>p</sub> , °C.       | 302     | 302     | 302     | 302     | 302     | 302     | 302    | 302     |
| CAP. (D × L), MILS         | 10 × 40 | 15 × 60 | 10 × 40 | 15 × 60 | 10 × 40 | 10 × 40 | 9 × 50 | 15 × 72 |
| NO. FILAMENTS              | 34      | 34      | 34      | 34      | 34      | 34      | 34     | 34      |
| DPF                        | 2.88    | 2.90    | 2.86    | 2.89    | 2.89    | 2.90    | 2.89   | 2.92    |
| SHAPE                      | RND     | RND     | RND     | RND     | RND     | RND     | RND    | TRI     |
| QUENCH                     | XF      | XF      | XF      | XF      | XF      | XF      | XF     | XF      |
| MODULUS, G/D               | 44.7    | 48.2    | 40.6    | 45.1    | 53.3    | 51.6    | 42.0   | 46.4    |
| ELNG. (E <sub>b</sub> ), % | 76.3    | 78.8    | 88.4    | 84.2    | 68.4    | 68.5    | 80.6   | 73.0    |
| TENACITY, G/D              | 3.12    | 3.23    | 3.04    | 3.07    | 3.34    | 3.32    | 3.15   | 2.88    |
| S <sub>1</sub> , %         | 13.8    | 5.4     | 9.2     | 4.8     | 13.1    | 5.5     | 30.0   | 4.7     |
| DHS, %                     | 9.0     | 4.4     | 7.1     | 4.3     | 9.4     | 4.5     | 24.6   | 4.0     |
| (DHS-S <sub>1</sub> ), %   | -4.8    | -1.0    | -2.1    | -0.5    | -3.7    | -1.0    | -5.5   | -0.7    |
| ST <sub>max</sub> , MG/D   | 91      | 85      | 52      | 65      | 87      | 92      | 73     | 72      |
| Ms, G/D                    | 0.60    | 1.57    | 0.57    | 1.35    | 0.66    | 1.67    | 0.53   | 1.53    |
| Ps, G/D                    | 1.26    | 0.46    | 0.48    | 0.31    | 1.14    | 0.51    | 1.01   | 0.34    |
| DENSITY, G/CC              | 1.353   | 1.359   | 1.353   | 1.356   | 1.351   | 1.356   | 1.348  | 1.359   |
| RDDR, x1000                | 120     | 98      | 145     | 139     | 109     | 99      | 119    | 147     |
| EX. XVI-                   | 9       | 10      | 11      | 12      | 13      | 14      | 15     |         |
| SPIN SPEED, YPM            | 4500    | 4500    | 4500    | 4500    | 4500    | 5500    | 5500   |         |
| SPIN SPEED, MPM            | 4115    | 4115    | 4115    | 4115    | 4115    | 5029    | 5029   |         |
| [n]                        | 0.65    | 0.65    | 0.65    | 0.65    | 0.65    | 0.65    | 0.65   |         |
| T <sub>p</sub> , °C.       | 302     | 296     | 296     | 302     | 302     | 305     | 297    |         |
| CAP. (D × L), MILS         | 15 × 72 | 9 × 50  | 15 × 72 | 10 × 40 | 15 × 60 | 9 × 50  | 9 × 36 |         |
| NO. FILAMENTS              | 34      | 68      | 34      | 40      | 34      | 34      | 34     |         |
| DPF                        | 4.34    | 2.22    | 3.06    | 2.45    | 2.90    | 5.20    | 4.90   |         |
| SHAPE                      | TRI     | RND     | OCTA    | RND     | RND     | RND     | RND    |         |
| QUENCH                     | XF      | 4RAD    | 2RAD    | XF      | XF      | 4XF     | XF     |         |
| MODULUS, G/D               | 43.4    | 36.9    | 51.1    | 43.8    | 48.2    | 53.3    | 45.6   |         |
| ELNG. (E <sub>b</sub> ), % | 73.8    | 87.0    | 71.4    | 78.8    | 78.8    | 60.8    | 65.8   |         |
| TENACITY, G/D              | 2.82    | 3.04    | 2.98    | 3.18    | 3.23    | 3.96    | 3.56   |         |
| S <sub>1</sub> , %         | 15.3    | 20.1    | 3.4     | 7.6     | 5.4     | 9.1     | 3.4    |         |
| DHS, %                     | 10.1    | 13.6    | 3.3     | 6.9     | 4.4     | 8.0     | 3.7    |         |
| (DHS-S <sub>1</sub> ), %   | -5.2    | -6.5    | -0.1    | -0.7    | -1.0    | -1.1    | 0.3    |         |
| ST <sub>max</sub> , MG/D   | 62      | 78      | 75      | 76      | 85      | 65      | 76     |         |
| Ms, G/D                    | 0.41    | 0.39    | 2.21    | 1.00    | 1.57    | 0.71    | 2.24   |         |
| Ps, G/D                    | 0.95    | 1.57    | 0.26    | 0.58    | 0.46    | 0.59    | 0.26   |         |
| DENSITY, G/CC              | 1.352   | 1.352   | 1.371   | 1.356   | 1.359   | 1.354   | 1.371  |         |
| RDDR, x1000                | 115     | 139     | 202     | 101     | 98      | N/A     | 100    |         |

TABLE XVII

| EX. XVII-                  | 1       | 2       | 3       | 4       | 5       | 6       | 7       | 8       | 9       |
|----------------------------|---------|---------|---------|---------|---------|---------|---------|---------|---------|
| YARN TYPE                  | 1-HIGH  | 1-LOW   | 1-MIX   | 2-HIGH  | 2-LOW   | 2-MIX   | 3-HIGH  | 3-LOW   | 3-MIX   |
| SPIN SPEED, YPM            | 4500    | 4500    | 4500    | 4500    | 4500    | 4500    | 4000    | 4000    | 4000    |
| SPIN SPEED, MPM            | 4115    | 4115    | 4115    | 4115    | 4115    | 4115    | 3658    | 3658    | 3658    |
| [n]                        | 0.65    | 0.65    | 0.65    | 0.65    | 0.65    | 0.65    | 0.65    | 0.65    | 0.65    |
| T <sub>p</sub> , °C.       | 302     | 302     | 302     | 302     | 302     | 302     | 288     | 288     | 288     |
| CAP. (D × L), MILS         | 9 × 50  | 15 × 72 | N/A     | 9 × 50  | 15 × 72 | N/A     | 9 × 12  | 15 × 60 | N/A     |
| NO. FILAMENTS              | 34 + 34 | 40 + 40 | 34 + 40 | 34 + 34 | 34 + 34 | 34 + 34 | 17 + 17 | 34 + 34 | 17 + 34 |
| DPF                        | 2.2     | 1.9     | N/A     | 2.2     | 2.2     | N/A     | 3.9     | 2.0     | N/A     |
| SHAPE                      | RND     | OCTA    | N/A     | RND     | TRI     | N/A     | RND     | RND     | RND     |
| QUENCH                     | XF      | XF      | XF      | XF      | XF      | XF      | XF      | XF      | XF      |
| MODULUS, G/D               | 43.3    | 53.8    | 50.5    | 43.4    | 49.7    | 49.7    | 30.9    | 38.6    | 28.8    |
| ELNG. (E <sub>b</sub> ), % | 82.0    | 80.9    | 76.6    | 82.0    | 71.7    | 72.7    | 98.0    | 90.0    | 102.0   |
| TENACITY, G/D              | 3.15    | 3.39    | 3.07    | 3.15    | 2.96    | 2.92    | 2.80    | 2.90    | 2.80    |
| S <sub>1</sub> , %         | 12.5    | 3.9     | 11.0    | 12.5    | 3.9     | 10.6    | 16.7    | 5.9     | 16.5    |
| DHS, %                     | 9.4     | 3.7     | 8.8     | 9.4     | 4.2     | 7.4     | 16.3    | 5.3     | 16.0    |
| (DHS-S <sub>1</sub> ), %   | -3.1    | -0.2    | -2.2    | -3.1    | 0.3     | -3.2    | -0.4    | -0.6    | -0.5    |
| ST <sub>max</sub> , MG/D   | 75      | 86      | 81      | 75      | 77      | 76      | 77      | 97      | 73      |
| Ms, G/D                    | 0.60    | 2.21    | 0.74    | 0.60    | 1.97    | 0.72    | 0.46    | 1.64    | 0.44    |
| Ps, G/D                    | 0.94    | 0.34    | 0.89    | 0.94    | 0.30    | 0.81    | 1.29    | 0.57    | 1.20    |
| DENSITY, G/CC              | 1.3514  | 1.3627  | 1.3570  | 1.3514  | 1.3620  | 1.3573  | 1.3484  | 1.3600  | 1.3561  |
| RDDR, x1000                | 119     | 126     | 123     | 119     | 139     | 129     | —       | —       | 195     |
| DFL (DHS), %               | 0.0     | 0.0     | 5.1     | 0.0     | 0.0     | 5.2     | 0.0     | 0.0     | 11.0    |
| REL. BULK, %               | 3.1     | 0.2     | 8.8     | 3.1     | 0.3     | 8.3     | 0.4     | 0.6     | 11.4    |

TABLE XVIII

| YARN TYPE | DRAWING MODE |           | HEAT TREATMENT |        | RELATIVE AGE |
|-----------|--------------|-----------|----------------|--------|--------------|
|           | A            | B (B1/B2) | A              | B      |              |
| Control   | ND           | ND        | NO             | NO     | A > B        |
| I         | N/A          | COLD/ND   | N/A            | NO/NO  | B1 > B2      |
| II        | N/A          | COLD/COLD | N/A            | NO/YES | B1 > B2      |
| III       | N/A          | COLD/HOT  | N/A            | NO/YES | B1 > B2      |
| IV        | N/A          | COLD/HOT  | N/A            | NO/NO  | B1 > B2      |
| V         | COLD         | COLD      | NO             | NO     | A > B        |
| VI        | COLD         | COLD      | NO             | NO     | A > B        |
| VII       | COLD         | COLD      | NO             | YES    | A > B        |
| VIII      | COLD         | HOT       | NO             | YES    | A > B        |
| IX        | COLD         | HOT       | NO             | NO     | A > B        |
| X         | COLD         | COLD      | YES            | NO     | B > A        |
| XI        | HOT          | COLD      | YES            | NO     | B > A        |
| XII       | HOT          | COLD      | NO             | NO     | B > A        |
| XIII      | COLD         | ND        | NO             | YES    | A > B        |
| XIV       | COLD         | ND        | NO             | NO     | A > B        |

ND = NO DRAW; N/A = NOT APPLICABLE

What is claimed is:

1. A process for improving the properties of a mixed shrinkage yarn of spin-oriented polyester filaments of elongation-to-break (E<sub>b</sub>) about 40 to about 120% comprised of polyester filaments (A<sub>F</sub>) of high boil-off shrinkage (S<sub>1</sub>) greater than about 15% and of low shrinkage polyester filaments (B<sub>F</sub>), wherein the mixed shrinkage yarn is cold-drawn without heat-setting to provide drawn filaments of elongation-to-break (E<sub>b</sub>) less than about 30% from drawing said filaments (A<sub>F</sub>) of high boil-off shrinkage, and wherein said low shrinkage filaments (B<sub>F</sub>) are of tenacity at 7% elongation (T<sub>7</sub>) at least about 0.7 grams/denier, boil-off shrinkage (S<sub>1</sub>) less than about 10%, thermal stability as shown by an (S<sub>2</sub>) value less than about +1%, net shrinkage (S<sub>12</sub>) less than about 8%, maximum shrinkage tension (ST) less than about 0.3 grams/denier, density ( $\rho$ ) about 1.35 to about 1.39 grams/cubic Centimeter, and crystal size (CS) about 55 to about 90 Angstroms and also at least about (250 $\rho$ -282.5) Angstroms.

2. A process according to claim 1, wherein said mixed shrinkage yarn is prepared by cospinning polyester filaments (A<sub>F</sub>) and (B<sub>F</sub>) and winding said mixed shrinkage yarn at a speed of at least 3.5 xm/min.

3. A process for preparing a mixed shrinkage yarn, 25 wherein spin-oriented polyester filaments (A<sub>F</sub>) of elongation-to-break (E<sub>b</sub>) about 40 to 120% and of high boil-off shrinkage (S<sub>1</sub>) greater than about 15% are cold-drawn without heat-setting to provide drawn filaments of elongation-to-break (E<sub>b</sub>) less than about 30%, and 30 spin-oriented low shrinkage polyester filaments (B<sub>F</sub>) are cold-drawn without heat setting and the filaments are co-mingled before or after drawing to form a mixed shrinkage yarn, and wherein said filaments (B<sub>F</sub>) are of elongation-to-break about 40 to about 120% tenacity at 35 7% elongation (T<sub>7</sub>) at least about 0.7 grams/denier, boil-off shrinkage (S<sub>1</sub>) less than about 10%, thermal stability as shown by an S<sub>2</sub> value less than about +1%, net shrinkage (S<sub>12</sub>) less than about 8%, maximum shrinkage tension (ST) less than about 0.3 grams/denier, 40 density ( $\rho$ ) about 1.35 to about 1.39 grams/cubic Centimeter, and crystal size (CS) about 55 to about 90 Angstroms and also at least about (250 $\rho$ -282.5) Angstroms.

4. A process for preparing a mixed shrinkage yarn, 45 wherein spin-oriented polyester filaments (A<sub>F</sub>) of high boil-off shrinkage (S<sub>1</sub>) greater than about 15% are cold drawn without post heat treatment, said drawing being carried out such that the elongation-to-break (E<sub>b</sub>) of the resulting drawn filaments is less than about 30%, and spin-oriented low shrinkage polyester filaments (B<sub>F</sub>) are 50 drawn hot, with or without post heat treatment, and the resulting drawn filaments are co-mingled to provide a mixed shrinkage yarn of uniformly drawn filaments, wherein said low shrinkage filaments (B<sub>F</sub>) are of elongation-to-break (E<sub>b</sub>) about 40 to about 120%, tenacity at 55 7% elongation (T<sub>7</sub>) at least about 0.7 grams/denier, boil-off shrinkage (S<sub>1</sub>) less than about 10%, thermal stability as shown by an S<sub>2</sub> value less than about +1%, net shrinkage (S<sub>12</sub>) less than about 8%, maximum shrinkage tension (ST) less than about 0.3 grams/denier, 60 density ( $\rho$ ) about 1.35 to about 1.39 grams/cubic centimeter, and crystal size (CS) about 55 to about 90 Angstrom and also at least about (250 $\rho$ -282.5) Angstroms.

5. A process for preparing a mixed shrinkage yarn, 65 wherein spin-oriented polyester filaments (A<sub>F</sub>) of high boil-off shrinkages (S<sub>1</sub>) greater than about 15% and spin-oriented low shrinkage polyester filaments (B<sub>F</sub>) are cold-drawn to form separate drawn filament bundles (A)<sub>D</sub> and (B)<sub>D</sub>, respectively, and such that the elonga-

tion-to-break ( $E_B$ ) of resulting drawn filament bundle ( $A_D$ ) is less than about 30%, and one bundle is heat set and co-mingled with the other bundle to provide a mixed shrinkage yarn of uniformly drawn polyester filaments, and wherein said low shrinkage filaments ( $B_F$ ) are of elongation-to-break ( $E_B$ ) about 40 to about 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter, and crystal size (CS) about 55 to about 90 Angstroms and also at least about (250 $\rho$ -282.5) Angstroms.

6. A process for preparing a mixed shrinkage yarn, wherein spin-oriented polyester filaments ( $A_F$ ) of high boil-off shrinkage ( $S_1$ ) greater than about 15% are drawn hot, with or without post heat treatment, such that the elongation-to-break ( $E_B$ ) of the resulting drawn filaments is less than about 30%, and spin-oriented low shrinkage polyester filaments ( $B_F$ ) are drawn cold, without post heat treatment, and the resulting drawn filaments are co-mingled to provide a mixed shrinkage yarn of uniformly drawn polyester filaments, wherein said low shrinkage filaments ( $B_F$ ) are of elongation-to-break ( $E_B$ ) about 40 to about 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter, and crystal size (CS) about 55 to about 90 Angstroms and also at least about (250 $\rho$ -282.5) Angstroms.

7. A process for preparing a mixed shrinkage yarn, wherein spin-oriented polyester filaments ( $A_F$ ) of high boil-off shrinkages ( $S_1$ ) greater than about 15% are cold-drawn with or without heat setting, said drawing being carried out such that the elongation-to-break ( $E_B$ ) of the resulting drawn filaments is less than about 30%, and co-mingled with spin-oriented low shrinkage polyester filaments ( $B_F$ ) to provide a mixed shrinkage yarn, and wherein said low shrinkage filaments ( $B_F$ ) are of elongation-to-break ( $E_B$ ) about 40 to 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter, and crystal size (CS) about 55 to about 90 Angstroms and also at least about (250 $\rho$ -282.5) Angstroms.

8. A process for preparing a mixed shrinkage yarn, wherein spin-oriented polyester filaments are cold-drawn, the resulting drawn filaments are separated into at least two filament bundles, only one of which bundles is heat set, and then the filament bundles are co-mingled to provide a mixed shrinkage yarn of uniformly drawn filaments, wherein said spin-oriented filaments are of elongation-to-break ( $E_B$ ) about 40 to about 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter, and crystal size (CS) about 55 to about 90 Angstroms and also at least about (250 $\rho$ -282.5) Angstroms.

9. A process for preparing a mixed shrinkage yarn from at least two bundles of low shrinkage spin-oriented polyester filaments, wherein one of said bundles is drawn cold without post heat treatment and another of said bundles is drawn hot or cold with post heat treatment, or drawn hot with post heat treatment, and the resulting drawn filaments are co-mingled to provide a mixed shrinkage yarn of uniformly drawn filaments, and wherein said spin-oriented filaments are of elongation-to-break ( $E_B$ ) about 40 to about 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter and crystal size (CS) about 55 to about 90 Angstroms and also at least about (250 $\rho$ -282.5) Angstroms.

10. A process for preparing a mixed shrinkage yarn from at least two bundles of low shrinkage spin-oriented polyester filaments, wherein one of said bundles is drawn hot with or without post heat treatment and the resulting drawn filaments are comingled with another of said bundles of spin-oriented filaments to provide a mixed shrinkage yarn, and wherein said spin-oriented filaments are of elongation-to-break ( $E_B$ ) about 40 to about 120%, tenacity at 7% elongation ( $T_7$ ) at least about 0.7 grams/denier, boil-off shrinkage ( $S_1$ ) less than about 10%, thermal stability as shown by an ( $S_2$ ) value less than about +1%, net shrinkage ( $S_{12}$ ) less than about 8%, maximum shrinkage tension (ST) less than about 0.3 grams/denier, density ( $\rho$ ) about 1.35 to about 1.39 grams/cubic centimeter and crystal size (CS) about 55 to about 90 Angstroms and also at least about (250 $\rho$ -282.5) Angstroms.

11. A process according to claim 7 or 10, wherein said spin-oriented filaments are filaments that have been processed with post heat treatment.

12. A process according to any one of claims 1 to 10, wherein the resulting mixed shrinkage yarn has a differential filament shrinkage of at least about 5% and a maximum shrinkage tension (ST) at least about 0.15 gpd.

13. A process according to any one of claims 1 to 10, wherein the drawing is carried out with the filaments in the form of a weftless warp sheet of filament bundles or yarns prior to knitting, weaving or winding onto a beam.

14. A process according to any one of claims 1 to 10, wherein the filaments or mixed shrinkage yarns are air jet-textured.

15. A process according to any one of claims 1 to 10, wherein the polyester of at least some of said filaments is modified with about 1 to about 3% by weight of ethylene-5-sodium-sulfo isophthalate.

16. A process according to claim 15, wherein such polyester contains a chainbranching agent in minor amount sufficient to provide boil-off shrinkage ( $S_1$ ) of less than about 10%.

17. A process according to any one of claims 1 to 10, wherein the resulting filaments of low shrinkage are of denier less than about one.

18. A process according to any one of claims 1 to 10, wherein the resulting mixed shrinkage yarn is relaxed by heat treatment to develop bulk on account of the difference in shrinkages and to form a bulky yarn.

19. A process according to claim 18, wherein a plurality of bundles of filaments having different shrinkages are relaxed to develop bulk and are in the form of a weftless warp sheet of filament bundles or yarns.

\* \* \* \* \*